



US005985531A

# United States Patent [19]

Nakamine et al.

[11] Patent Number: 5,985,531

[45] Date of Patent: Nov. 16, 1999

[54] SILVER HALIDE COLOR PHOTOGRAPHIC LIGHT-SENSITIVE MATERIAL CONTAINING A DEVELOPMENT INHIBITOR RELEASING COMPOUND

[75] Inventors: **Takeshi Nakamine; Hajime Nakagawa; Osamu Uchida; Hideaki Sato; Toshio Kawagishi**, all of Minami-Ashigara, Japan

[73] Assignee: **Fuji Photo Film Co., Ltd.**, Kanagawa, Japan

[21] Appl. No.: 08/887,931

[22] Filed: Jul. 3, 1997

## [30] Foreign Application Priority Data

Jul. 8, 1996 [JP] Japan ..... 8-195239  
Jul. 2, 1997 [JP] Japan ..... 9-190767

[51] Int. Cl. <sup>6</sup> ..... G03C 7/305

[52] U.S. Cl. ..... 430/544; 430/957

[58] Field of Search ..... 430/544, 957

## [56] References Cited

### U.S. PATENT DOCUMENTS

5,326,680 7/1994 Ohkawa et al.  
5,630,927 5/1997 Kawagishi et al. ..... 430/544

### FOREIGN PATENT DOCUMENTS

7133259 5/1995 Japan.

Primary Examiner—Janet Baxter

Assistant Examiner—Amanda C. Walke

Attorney, Agent, or Firm—Birch, Stewart, Kolasch & Birch, LLP

## [57] ABSTRACT

A silver halide color photographic light-sensitive material containing a compound represented by formula (I) below formula (I)



wherein A represents a coupler residue, X<sub>1</sub> represents a heterocyclic group or a —C(X<sub>4</sub>)(X<sub>5</sub>)—Y group, Y represents an —SO<sub>2</sub>R<sup>1</sup>, —SO<sub>2</sub>NR<sup>1</sup>R<sup>2</sup>, —CONR<sup>1</sup>R<sup>2</sup>, —CO<sub>2</sub>Z, —CN, —CF<sub>3</sub>, —CCl<sub>3</sub>, or —NO<sub>2</sub> group, each of R<sup>1</sup> and R<sup>2</sup> independently represents a hydrogen atom or a substituted or nonsubstituted alkyl, cycloalkyl, alkenyl, aryl, or heterocyclic group, Z represents a hydrogen atom or a substituted or nonsubstituted cycloalkyl, alkenyl, aryl, or heterocyclic group, each of X<sub>2</sub>, X<sub>3</sub>, X<sub>4</sub>, and X<sub>5</sub> represents a hydrogen atom or a substituent group, and DI represents a development inhibitor residue which is bonded by a hetero atom and released to form mercaptoazole.

**16 Claims, No Drawings**

**SILVER HALIDE COLOR PHOTOGRAPHIC  
LIGHT-SENSITIVE MATERIAL  
CONTAINING A DEVELOPMENT  
INHIBITOR RELEASING COMPOUND**

**BACKGROUND OF THE INVENTION**

The present invention relates to a silver halide color photographic light-sensitive material containing a novel compound capable of releasing a development inhibitor with a high development inhibiting capacity at an appropriate timing during development.

Recently, as silver halide light-sensitive materials, particularly color light-sensitive materials for photographing, high-speed light-sensitive materials which are superior in graininess, sharpness, and color reproduction and also have a high storage stability are desired. One representative example is an ISO 400 light-sensitive material (Super G-400) having a high image quality equivalent to that of ISO 100.

As a compound which improves the sharpness and does not degrade the storage stability of a light-sensitive material, compounds which imagewise release a development inhibitor via two or more timing groups are described in, e.g., Jpn. Pat. Appln. KOKAI Publication Nos. 60-218645, 60-249148, and 61-156127 and U.S. Pat. No. 4,861,701. However, when any of these compounds is used, the speed (timing) at which the development inhibitor is released or the diffusibility of the development inhibitor is inappropriate. Therefore, the sharpness, graininess, and color reproduction are not satisfactorily improved. Also, many light-sensitive materials containing these compounds significantly increase the fog or decrease the sensitivity when left to stand for long time periods after exposure and before development or when exposed to a high-temperature, high-humidity ambient.

Jpn. Pat. Appln. KOKAI Publication No. 5-313322 has disclosed novel development inhibitor release compounds which can solve these problems. However, the disclosed practical compounds cannot meet recent increasing demands on image quality and are desired to be further improved.

**BRIEF SUMMARY OF THE INVENTION**

It is an object of the present invention to provide a silver halide color photographic light-sensitive material superior in sharpness, graininess, and color reproduction.

The above object is achieved by a silver halide color photographic light-sensitive material containing a compound represented by formula (I) below.

Formula (I)



wherein A represents a coupler residue,  $X_1$  represents a heterocyclic group or a  $-C(X_4)(X_5)-Y$  group, Y represents an  $-SO_2R^1$ ,  $-SO_2NR^1R^2$ ,  $-CONR^1R^2$ ,  $-CO_2Z$ ,  $-CN$ ,  $-CF_3$ ,  $-CCl_3$ , or  $-NO_2$  group, each of  $R^1$  and  $R^2$  independently represents a hydrogen atom or a substituted or nonsubstituted alkyl, cycloalkyl, alkenyl, aryl, or heterocyclic group, Z represents a hydrogen atom or a substituted or nonsubstituted cycloalkyl, alkenyl, aryl, or heterocyclic group, each of  $X_2$ ,  $X_3$ ,  $X_4$ , and  $X_5$  represents a hydrogen atom or a substituent group, and DI represents a development inhibitor residue which is bonded by a hetero atom and released to form mercaptoazole.

**DETAILED DESCRIPTION OF THE  
INVENTION**

The present invention will be described in more detail below.

Details of a compound represented by formula (I) will be described.

In formula (I), A represents a coupler residue and, more specifically, represents a yellow image forming coupler residue, a magenta image forming coupler residue, a cyan image forming coupler residue, a non-dye-forming coupler residue, or a dye release coupler residue. Details of these coupler residues are described in Research Disclosure No. 37038 (February, 1995), pages 80 to 85 and 87 to 89.

When A represents a yellow image forming coupler residue, examples are pivaloylacetanilide type, benzoylacetanilide type, malondiester type, malondiamide type, dibenzoylmethane type, benzothiazolylacetamide type, malonestermonoamide type, benzoxazolylacetamide type, benzoimidazolylacetamide type, benzothiazolylacetamide type, cycloalkanoylacetamide type, and indoline-2-ylacetamide type coupler residues, quinazoline-4-one-2-ylacetamide type coupler residues described in U.S. Pat. No. 5,021,332, benzo-1,2,4-thiadiazine-1,1-dioxide-3-ylacetamide type coupler residues described in U.S. Pat. No. 5,021,330, coupler residues described in European Patent No. 421221A, coupler residues described in U.S. Pat. No. 5,455,149, and coupler residues described in European Patent No. 0622673.

When A represents a magenta image forming coupler residue, examples are 5-pyrazolone type, 1H-pyrazolo[1,5-a]benzimidazole type, 1H-pyrazolo[5,1-c][1,2,4]triazole type, 1H-pyrazolo[1,5-b][1,2,4]triazole type, 1H-imidazo[1,2-b]pyrazole type, and cyanoacetophenone type coupler residues, active propene type coupler residues described in WO 93/01523, enamine type coupler residues described in WO 93/07534, 1H-imidazo[1,2-b][1,2,4]triazole type coupler residues, and coupler residues described in U.S. Pat. No. 4,871,652.

When A represents a cyan image forming coupler residues, examples are phenol type and naphthol type coupler residues, 2,5-diphenylimidazole type coupler residues described in European Patent No. 249453, 1H-pyrrolo[1,2-b][1,2,4]triazole type and 1H-pyrrolo[2,1-c][1,2,4]triazole type coupler residues, pyrrole type coupler residues described in Jpn. Pat. Appln. KOKAI Publication Nos. 4-188137 and 4-190347, 3-hydroxypyridine type coupler residues described in Jpn. Pat. Appln. KOKAI Publication No. 1-315736, pyrrolopyrazole type coupler residues described in U.S. Pat. No. 5,164,289, pyrroloimidazole type coupler residues described in Jpn. Pat. Appln. KOKAI Publication No. 4-174429, pyrazolopyrimidine type coupler residues described in U.S. Pat. No. 4,950,585, pyrrolotriazine type coupler residues described in Jpn. Pat. Appln. KOKAI Publication No. 4-204730, coupler residues described in U.S. Pat. No. 4,746,602, coupler residues described in U.S. Pat. No. 5,104,783, coupler residues described in U.S. Pat. No. 5,162,196, and coupler residues described in European Patent No. 0556700.

A can also be a coupler residue which does not essentially leave any color image. Examples of coupler residues of this sort are indanone type and acetophenone type coupler residues and elution type coupler residues described in European Patent Nos. 443530A and 444501A and Jpn. Pat. Appln. KOKAI Publication Nos. 6-138612, 6-82995, 6-82996, and 6-82998.

Preferable examples of a coupler residue represented by A in formula (I) are coupler residues represented by formulas (Cp-1), (Cp-2), (Cp-3), (Cp-4), (Cp-5), (Cp-6), (Cp-7), (Cp-8), (Cp-9), (Cp-10), (Cp-11), and (Cp-12). These couplers are preferable because of their high coupling speeds.



-continued

(Cp-1)



(Cp-2)



(Cp-3)

10

(Cp-4)



(Cp-5)

20



(Cp-6)

30



(Cp-7)

35

In the above formulas, a free bonding hand stemming from a coupling position represents the bonding position of  $-\text{O---C}(=\text{O})-\text{N}(\text{X}_1)-\text{C}(\text{X}_2)(\text{X}_3)-\text{DI}$  in formula (I).

In the above formulas, if  $\text{R}_{51}, \text{R}_{52}, \text{R}_{53}, \text{R}_{54}, \text{R}_{55}, \text{R}_{56}, \text{R}_{57}, \text{R}_{58}, \text{R}_{59}, \text{R}_{60}, \text{R}_{61}, \text{R}_{62}, \text{R}_{63}, \text{R}_{64}, \text{R}_{65}, \text{or R}_{66}$  includes a nondiffusion group, this group is so selected that the total number of carbon atoms is 8 to 40, preferably 10 to 30. In other cases, the total number of carbon atoms is preferably 15 or less. In a bis, telomer, or polymer type coupler, any of the above substituent groups represents a divalent group and connects a repeating unit or the like. If this is the case, the number of carbon atoms can fall outside the defined range.

$\text{R}_{51}$  to  $\text{R}_{66}$ , a, b, d, e, and f will be described in detail below.

50 In the present invention, "substituent groups" include the following groups. Examples of the "substituent groups" are a halogen atom (e.g., a fluorine atom, a chlorine atom, and a bromine atom), an alkyl group (preferably a 1- to 40-carbon, straight-chain or branched-chain alkyl group,

55 e.g., methyl, ethyl, propyl, isopropyl, butyl, t-butyl, 1-octyl, and tridecyl), a cycloalkyl group (preferably a 3- to 40-carbon cycloalkyl group, e.g., cyclopropyl, 1-ethylcyclopropyl, cyclopentyl, cyclohexyl, 1-norbornyl, and 1-adamantyl), an alkenyl group (preferably a 2- to

60 40-carbon alkenyl group, e.g., vinyl, allyl, and 3-butene-1-yl), an aryl group (preferably a 6- to 32-carbon aryl group, e.g., phenyl, 1-naphthyl, and 2-naphthyl), a heterocyclic group (preferably a 1- to 32-carbon, 5- to 8-membered heterocyclic group, e.g., 2-thienyl, 4-pyridyl, 2-furyl,

65 2-pyrimidinyl, 1-pyridyl, 2-benzothiazolyl, 1-imidazolyl, 1-pyrazolyl, and benzotriazole-2-yl), a cyano group, a silyl

group (preferably a 3- to 40-carbon silyl group, e.g., trimethylsilyl, triethylsilyl, tributylsilyl, t-butyldimethylsilyl, and t-hexyldimethylsilyl), a hydroxyl group, a carboxyl group, a nitro group, an alkoxy group (preferably a 1- to 40-carbon alkoxy group, e.g., methoxy, ethoxy, 1-butoxy, 2-butoxy, isopropoxy, t-butoxy, and dodecyloxy), a cycloalkyloxy group (preferably a 3- to 8-carbon cycloalkyl group, e.g., cyclopentyloxy and cyclohexyloxy), an aryloxy group (preferably a 6- to 40-carbon aryloxy group, e.g., phenoxy and 2-naphthoxy), a heterocyclic oxy group (preferably a 1- to 40-carbon heterocyclic oxy group, e.g., 1-phenyltetrazole-5-oxy, 2-tetrahydropyranloxy, and 2-furyloxy), a silyloxy group (preferably a 1- to 40-carbon silyloxy group, e.g., trimethylsilyloxy, t-butyldimethylsilyloxy, and diphenylmethylsilyloxy), an acyloxy group (preferably a 2- to 40-carbon acyloxy group, e.g., acetoxy, pivaloxy, benzoxyloxy, and dodecanoyloxy), an alkoxy carbonyloxy group (preferably a 2- to 40-carbon alkoxy carbonyloxy group, e.g., ethoxycarbonyloxy and t-butoxycarbonyloxy), a cycloalkyloxy carbonyloxy group (preferably a 4- to 40-carbon cycloalkyloxy carbonyloxy group, e.g., cyclohexyloxy carbonyloxy), an aryloxy carbonyloxy group (preferably a 7- to 40-carbon aryloxy carbonyloxy group, e.g., phenoxy carbonyloxy), a carbamoyloxy group (preferably a 1- to 40-carbon carbamoyloxy group, e.g., N,N-dimethylcarbamoyloxy and N-butylcarbamoyloxy), a sulfamoyloxy group (preferably a 1- to 40-carbon sulfamoyloxy group, e.g., N,N-diethylsulfamoyloxy and N-propylsulfamoyloxy), an alkanesulfonyloxy group (preferably a 1- to 40-carbon alkanesulfonyloxy group, e.g., methanesulfonyloxy and hexadecanesulfonyloxy), an arenesulfonyloxy group (preferably a 6- to 40-carbon arenesulfonyloxy group, e.g., benzenesulfonyloxy), an acyl group (preferably a 1- to 40-carbon acyl group, e.g., formyl, acetyl, pivaloyl, benzoyl, and tetradecanoyl), an alkoxy carbonyl group (preferably a 2- to 40-carbon alkoxy carbonyl group, e.g., methoxycarbonyl, ethoxycarbonyl, and octadecyloxycarbonyl), a cycloalkyloxy carbonyl group (preferably a 4- to 40-carbon cycloalkyloxy carbonyl group, e.g., cyclohexyloxy carbonyl), an aryloxy carbonyl group (preferably a 7- to 40-carbon aryloxy carbonyl group, e.g., phenoxy carbonyl), a carbamoyl group (preferably a 1- to 40-carbon carbamoyl group, e.g., carbamoyl, N,N-dibutylcarbamoyl, N-ethyl-N-octylcarbamoyl, and N-propylcarbamoyl), an amino group (preferably an amino group having 32 or less carbon atoms, e.g., amino, methylamino, N,N-diethylamino, tetradecylamino, and octadecylamino), an anilino group (preferably a 6- to 40-carbon anilino group, e.g., anilino and N-methylanilino), a heterocyclic amino group (preferably a 1- to 40-carbon heterocyclic amino group, e.g., 4-pyridylamino), a carbonamide group (preferably a 2- to 40-carbon carbonamide group, e.g., acetamide, benzamide, and tetradecaneamide), a ureido group (preferably a 1- to 40-carbon ureido group, e.g., ureido, N,N-dimethylureido, and N-phenylureido), an imide group (preferably an imide group having 10 or less carbon atoms, e.g., N-succinimide and N-phthalimide), an alkoxy carbonylamino group (preferably a 2- to 40-carbon alkoxy carbonylamino group, e.g., methoxycarbonylamino, ethoxycarbonylamino, t-butoxycarbonylamino, and octadecyloxycarbonylamino), a cycloalkyloxy carbonylamino group (preferably a 4- to 40-carbon cycloalkyloxy carbonylamino group, e.g., cyclohexyloxy carbonylamino), an aryloxy carbonylamino group (preferably a 7- to 40-carbon aryloxy carbonylamino group, e.g., phenoxy carbonylamino), a sulfonamide group (preferably a 1- to 40-carbon sulfonamide group, e.g., methanesulfonamide, butanesulfonamide, benzenesulfonamide, and hexadecanesulfonamide), a sulfamoylamino group (preferably a 1- to 40-carbon sulfamoylamino group, e.g., N,N-dipropylsulfamoylamino and N-ethyl-N-dodecylsulfamoylamino), an azo group (preferably a 1- to 40-carbon azo group, e.g., phenylazo), an alkylthio group (preferably a 1- to 40-carbon alkylthio group, e.g., ethylthio and octylthio), a cycloalkylthio group (preferably a 3- to 40-carbon cycloalkylthio group, e.g., cyclohexylthio), an arylthio group (preferably a 6- to 40-carbon arylthio group, e.g., phenylthio), a heterocyclic thio group (preferably a 1- to 40-carbon heterocyclic thio group, e.g., 2-benzothiazolylthio, 2-pyridylthio, and 1-phenyltetrazolylthio), an alkylsulfinyl group (preferably a 1- to 40-carbon alkylsulfinyl group, e.g., dodecanesulfinyl), an arenesulfinyl group (preferably a 6- to 40-carbon arenesulfinyl group, e.g., benzenesulfinyl), an alkanesulfonyl group (preferably a 1- to 40-carbon alkanesulfonyl group, e.g., methanesulfonyl and octanesulfonyl), an arenesulfonyl group (preferably a 6- to 40-carbon arenesulfonyl group, e.g., benzenesulfonyl and 1-naphthalenesulfonyl), an alkoxysulfonyl group (preferably a 1- to 40-carbon alkoxysulfonyl group, e.g., methoxysulfonyl and ethoxysulfonyl), a cycloalkyloxy sulfonyl group (preferably a 3- to 40-carbon cycloalkyloxy sulfonyl group, e.g., cyclopropyloxysulfonyl), an aryloxysulfonyl group (preferably a 6- to 40-carbon aryloxysulfonyl group, e.g., phenoxy sulfonyl and p-methylphenoxy sulfonyl), a sulfamoyl group (preferably a sulfamoyl group having 32 or less carbon atoms, e.g., sulfamoyl, N,N-dipropylsulfamoyl, and N-ethyl-N-dodecylsulfamoyl), a sulfo group, a phosphonyl group (preferably a 1- to 40-carbon phosphonyl group, e.g., phenoxy phosphonyl, octyloxy phosphonyl, and phenyl phosphonyl), and a phosphinoylamino group (diethoxy phosphinoylamino and dioctyloxy phosphinoylamino).

Substituent groups  $R_{51}$  to  $R_{66}$  and a, b, d, e, and f in formulas (Cp-1) to (Cp-12) will be described in more detail below.

In formula (Cp-1),  $R_{51}$  represents an alkyl group, a cycloalkyl group, an aryl group, or a heterocyclic group. a represents 0 or 1.  $R_{52}$  represents a hydrogen atom, an alkyl group, a cycloalkyl group, an aryl group, or a heterocyclic group.

In formula (Cp-2),  $R_{51}$  represents an alkyl group, a cycloalkyl group, an aryl group, or a heterocyclic group, each of  $R_{52}$  and  $R_{53}$  independently represents a hydrogen atom, an alkyl group, a cycloalkyl group, an aryl group, or a heterocyclic group, and b represents 0 or 1.

In formula (Cp-3),  $R_{54}$  represents an alkyl group, a cycloalkyl group, an aryl group, a heterocyclic group, a carbonamide group, a sulfonamide group, an amino group, an anilino group, an alkylthio group, an arylthio group, an alkoxy group, a cycloalkyloxy group, an aryloxy group, a ureido group, or an alkoxy carbonylamino group.  $R_{55}$  represents an alkyl group, a cycloalkyl group, an aryl group, or a heterocyclic group.

In formulas (Cp-4) and (Cp-5), each of  $R_{56}$  and  $R_{57}$  independently represents a hydrogen atom, an alkyl group, a cycloalkyl group, an aryl group, a heterocyclic group, a carbonamide group, a sulfonamide group, an amino group, an anilino group, an alkylthio group, cycloalkylthio group, an arylthio group, an alkoxy group, a ureido group, an aryloxy group, a cycloalkyloxy group, an alkoxy carbonylamino group, or a cycloalkyloxy carbonylamino group.

In formulas (Cp-6) and (Cp-7), each of  $R_{58}$  and  $R_{60}$  independently represents an alkyl group, a cycloalkyl group, an aryl group, or a heterocyclic group,  $R_{59}$  represents an alkyl group, a cycloalkyl group, an aryl group, a heterocyclic group, a silyl group, a carbonamide group, a sulfonamide group, an amino group, an anilino group, an alkylthio group, a cycloalkylthio group, an arylthio group, an alkoxy group, a cycloalkyloxy group, an aryloxy group, a ureido group, an alkoxy carbonylaminogroup, a cycloalkyloxycarbonylaminogroup, or a halogen atom, and  $d$  represents any integer from 0 to 3. If  $d$  is a plural number, a plurality of  $R_{59}$ 's represent the same substituent group or different substituent groups.

In formula (Cp-8),  $R_{61}$  represents an alkyl group, a cycloalkyl group, an aryl group, a heterocyclic group, a carbamoyl group, an alkoxy carbonyl group, a cycloalkyloxycarbonyl group, an aryloxy carbonyl group, a cyano group, a sulfamoyl group, a carbonamide group, a ureido group, an alkoxy carbonylaminogroup, a cycloalkyloxycarbonylaminogroup, an aryloxy carbonylaminogroup, or a sulfonamide group,  $R_{62}$  represents an alkyl group, a cycloalkyl group, an aryl group, a heterocyclic group, a carbonamide group, a sulfonamide group, an amino group, an anilino group, an alkylthio group, a cycloalkylthio group, an arylthio group, an alkoxy group, a cycloalkyloxy group, an aryloxy group, a ureido group, an alkoxy carbonylaminogroup, a cycloalkyloxycarbonylaminogroup, or a halogen atom, and  $e$  represents any integer from 0 to 4. If  $e$  is a plural number, a plurality of  $R_{62}$ 's represent the same group or different groups.

In formulas (Cp-9) and (Cp-10),  $R_{63}$  represents an alkyl group, a cycloalkyl group, an aryl group, a heterocyclic group, a carbonamide group, a sulfonamide group, an amino group, an anilino group, an alkylthio group, a cycloalkylthio group, an arylthio group, an alkoxy group, a cycloalkyloxy group, an aryloxy group, a ureido group, an alkoxy carbonylaminogroup, a cycloalkyloxycarbonylaminogroup, or a halogen atom,  $e$  represents any integer from 0 to 4, and  $f$  represents any integer from 0 to 2. If  $e$  or  $f$  is a plural number, a plurality of  $R_{63}$ 's represent the same group or different groups.

In formulas (Cp-11) and (Cp-12), each of  $R_{64}$  and  $R_{65}$  independently represents a carbamoyl group, an alkoxy carbonyl group, a cycloalkyloxycarbonyl group, an aryloxy carbonyl group, a cyano group, a sulfamoyl group, an alkane sulfonyl group, an arenesulfonyl group, or a nitro group, and  $R_{66}$  represents a hydrogen atom, an alkyl group, a cycloalkyl group, an aryl group, or a heterocyclic group.

The numbers of carbon atoms and practical examples of the groups enumerated above in the explanation of substituent groups  $R_{51}$  to  $R_{66}$  are the same as those of the "substituent groups" described previously. Groups represented by  $R_{51}$  to  $R_{66}$  can further have substituent groups. Preferable examples of the substituent groups are a halogen atom, an alkyl group, a cycloalkyl group, an alkenyl group, an aryl group, a heterocyclic group, a cyano group, a silyl group, a hydroxyl group, a carboxyl group, a nitro group, an alkoxy group, a cycloalkyloxy group, an aryloxy group, a heterocyclic oxy group, a silyloxy group, an acyloxy group, an alkoxy carbonyloxy group, a cycloalkyloxycarbonyloxy group, an aryloxy carbonyloxy group, a carbamoyloxy group, a sulfamoyloxy group, an alkanesulfonyloxy group, an arenesulfonyloxy group, an acyl group, an alkoxy carbonyl group, a cycloalkyloxycarbonyl group, an aryloxy carbonyl group, a carbamoyl group, an amino group, an anilino group, a heterocyclic amino group, a carbonamide group, an alkoxy carbonylaminogroup, a cycloalkyloxycarbonylaminogroup, or a halogen atom, and  $d$  be 1 or 2.

5 lamino group, an aryloxycarbonylaminogroup, a ureido group, a sulfonamide group, a sulfamoylaminogroup, an imide group, an alkylthio group, an arylthio group, a heterocyclic thio group, a sulfinyl group, a sulfo group, an alkanesulfonyl group, an arenesulfonyl group, a sulfamoyl group, a phosphonyl group, and a phosphinoylaminogroup. Preferable carbon numbers and practical examples of these groups are the same as those of the above-mentioned "substituent groups". The substituent groups of groups represented by  $R_{51}$  to  $R_{66}$  are more preferably a halogen atom, an alkyl group, a cycloalkyl group, an aryl group, a silyl group, a hydroxyl group, a carboxyl group, an alkoxy group, a cycloalkyloxy group, an aryloxy group, an alkoxy carbonyl group, a cycloalkyloxycarbonyl group, a carbamoyl group, a carbonamide group, an alkoxy carbonylaminogroup, a cycloalkyloxycarbonylaminogroup, an aryloxy carbonylaminogroup, a sulfonamide group, an imide group, an alkylthio group, a cycloalkylthio group, an arylthio group, an alkanesulfonyl group, an arenesulfonyl group, a phosphonyl group, and a phosphinoylaminogroup.

10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630

In formula (Cp-8), it is preferable that  $R_{61}$  be a heterocyclic group, a carbamoyl group, an alkoxy carbonyl group, a cycloalkyloxy carbonyl group, an aryloxy carbonyl group, a cyano group, a sulfamoyl group, a carbonamide group, a ureido group, an alkoxy carbonylamino group, a cycloalkyloxy carbonyl group, an aryloxy carbonylamino group, or a sulfonamide group,  $R_{62}$  be a carbonamide group, a sulfonamide group, a ureido group, an alkoxy carbonylamino group, a cycloalkyloxy carbonyl group, or a halogen atom, and  $e$  be any integer from 0 to 2. It is more preferable that  $R_{61}$  be a carbamoyl group or a sulfamoyl group,  $R_{62}$  be a carbonamide group, a ureido group, or an alkoxy carbonylamino group, and  $e$  be 0 or 1.

In formulas (Cp-9) and (Cp-10), it is preferable that  $R_{63}$  be an alkyl group, a cycloalkyl group, an aryl group, a carbonamide group, a sulfonamide group, an alkylthio group, a cycloalkylthio group, an arylthio group, an alkoxy group, a cycloalkyloxy group, an aryloxy group, a ureido group, an alkoxy carbonylamino group, or a cycloalkyloxy carbonylamino group,  $e$  be 1 or 2, and  $f$  be 1 or 2.

In formulas (Cp-11) and (Cp-12), it is preferable that  $R_{64}$  be a cyano group, a carbamoyl group, an alkoxy carbonyl group, a cycloalkyloxy carbonyl group, or an aryloxy carbonyl group,  $R_{65}$  be a carbamoyl group, an alkoxy carbonyl group, a cycloalkyloxy carbonyl group, an aryloxy carbonyl group, or a cyano group, and  $R_{66}$  be an alkyl group, a cycloalkyl group, or an aryl group. It is more preferable that  $R_{64}$  be a cyano group,  $R_{65}$  be an alkoxy carbonyl group, a cycloalkyloxy carbonyl group, or an aryloxy carbonyl group, and  $R_{66}$  be an alkyl group, a cycloalkyl group, or an aryl group.

Preferable carbon numbers and practical examples of the preferable ranges of  $R_{51}$  to  $R_{66}$  and  $a, b, d, e$ , and  $f$  are the same as those of the above-mentioned "substituent groups".

In formula (I),  $X_1$  represents a heterocyclic group (the same as those of the above-mentioned "substituent groups") or a  $—C(X_4)(X_5)Y$  group.

$Y$  represents an  $—SO_2R^1$ ,  $—SO_2NR^1R^2$ ,  $—CONR^1R^2$ ,  $—CO_2Z$ ,  $—CN$ ,  $—CF_3$ ,  $—CCl_3$ , or  $—NO_2$  group.

Each of  $R^1$  and  $R^2$  independently represents a hydrogen atom or a substituted or nonsubstituted alkyl, cycloalkyl, alkenyl, aryl, or heterocyclic group, each of which has the same meaning as defined in the explanation of the above-mentioned "substituent groups". When  $R^1$  and  $R^2$  have substituent groups, these substituent groups are the same as those of the above-mentioned "substituent groups".  $R^1$  and  $R^2$  can also bond to each other to form a nitrogen-containing ring.

Each of  $R^1$  and  $R^2$  is independently preferably a hydrogen atom or a substituted or nonsubstituted alkyl group, and more preferably a hydrogen atom or an alkyl group which has a hydroxyl group and/or a carboxyl group as a substituent group and has 10 or less carbon atoms.

Preferable carbon numbers and practical examples of these preferable  $R^1$  and  $R^2$  are the same as those of the above-mentioned "substituent groups".

$Z$  represents a hydrogen atom or a substituted or nonsubstituted cycloalkyl, alkenyl, aryl, or heterocyclic group, each of which has the same meaning as that of the above-mentioned "substituent groups". When  $Z$  has a substituent group, this substituent group is any of the groups enumerated as the above-mentioned "substituent groups".

$Z$  is preferably a hydrogen atom or a substituted or nonsubstituted aryl group, and more preferably a hydrogen atom or a substituted aryl group having 10 or less carbon

atoms. Preferable substituent groups are a halogen atom, a hydroxyl group, and a carboxyl group.

$Y$  is preferably  $—CONR^1R^2$ ,  $—CO_2Z$ ,  $—CN$ , or  $—CF_3$ , and most preferably  $—CN$ .

Each of  $X_2$ ,  $X_3$ ,  $X_4$ , and  $X_5$  represents a hydrogen atom or a substituent group. This substituent group is the same as those of the above-mentioned "substituent groups" and can also be further substituted by the groups enumerated above as the "substituent groups".

Each of  $X_2$ ,  $X_3$ ,  $X_4$ , and  $X_5$  is preferably a hydrogen atom or a substituted or nonsubstituted alkyl or aryl group, and most preferably a hydrogen atom.

Preferable carbon numbers and practical examples of these preferable  $X_2$ ,  $X_3$ ,  $X_4$ , and  $X_5$  are the same as those of the above-mentioned "substituent groups".

A compound represented by formula (I) of the present invention is particularly preferably represented by formula (II) below.

Formula (II)



wherein each of  $A$ ,  $Y$ , and  $DI$  has the same meaning as defined in the explanation of formula (I).

Preferable practical examples of a partial structure represented by  $—N(X_1)—C(X_2)(X_3)Y$  in formula (I) will be presented below, but the present invention is not limited to these examples.



11



12



DJ-1



DL-2



DL-3



DL-4

In the above formula, examples of  $R_{91}$  are a halogen atom (e.g., a bromine atom and a chlorine atom), an alkyl group (a 1- to 20-carbon, preferably 1- to 10-carbon, straight-chain or branched-chain alkyl group, e.g., methyl, ethyl, butyl, t-butyl, neopentyl, t-amyl, propyloxycarbonylmethyl, butoxycarbonylethyl, 4-methoxybenzyl, and benzyl), a cycloalkyl group (a 3- to 20-carbon, preferably 3- to 10-carbon cycloalkyl group, e.g., cyclopropyl, 1-ethylcyclopropyl, cyclopentyl, cyclohexyl, 1-norbornyl, and 1-adamantyl), an aryl group (a 6- to 20-carbon, preferably 6- to 15-carbon aryl group, e.g., phenyl, naphthyl, 4-hydroxyphenyl, 3-methoxycarbonylphenyl, and 4-ethoxycarbonylphenyl), a heterocyclic group (a 1- to 20-carbon, preferably 1- to 12-carbon, monocyclic or condensed-ring heterocyclic group which contains at least one nitrogen, oxygen, or sulfur atom as a hetero atom and is preferably a 5- or 6-membered ring, e.g., 2-pyridyl, 2-furyl, 1-pyrrolyl, morpholino, and 1-indoliny), an alkoxy group (a 1- to 20-carbon, preferably 1- to 10-carbon alkoxy group, e.g., methoxy, ethoxy, and benzyloxy), a cycloalkyloxy group (a 3- to 20-carbon, preferably 3- to 10-carbon cycloalkyloxy group, e.g., cyclopropyloxy, 1-ethylcyclopropyloxy, cyclopentyloxy, and cyclohexyloxy), an aryloxy group (a 6- to 20-carbon, preferably 6- to 10-carbon aryloxy group, e.g., phenoxy, 4-methoxyphenoxy, and naphthoxy), a heterocyclic oxy group (preferably a 1- to 10-carbon heterocyclic oxy group, e.g., 1-phenyltetrazole-5-oxy, 2-tetrahydropyranloxy, and 2-furyloxy), a silyloxy group (preferably a 1- to 12-carbon silyloxy group, e.g., trimethylsilyloxy, t-butylidimethylsilyloxy, and diphenylmethylsilyloxy), an acyloxy group (preferably a 2- to 10-carbon acyloxy group, e.g., acetoxy, pivaloyloxy, benzyloxy, and dodecanoyloxy), an alkoxy carbonyloxy group (preferably a 2- to 10-carbon

alkoxycarbonyloxy group, e.g., ethoxycarbonyloxy and t-butoxycarbonyloxy), a cycloalkyloxycarbonyloxy group (preferably a 4- to 10-carbon cycloalkyloxycarbonyloxy group, e.g., cyclohexyloxycarbonyloxy), an aryloxycarbonyloxy group (preferably a 7- to 12-carbon aryloxycarbonyloxy group, e.g., phenoxy carbonyloxy), a carbamoyloxy group (preferably a 1- to 10-carbon carbamoyloxy group, e.g., N,N-dimethyl carbamoyloxy and N-butyl carbamoyloxy), a sulfamoyloxy group (preferably a 1- to 10-carbon sulfamoyloxy group, e.g., N,N-diethyl sulfamoyloxy and N-propyl sulfamoyloxy), an alkanesulfonyloxy group (preferably a 1- to 10-carbon alkanesulfonyloxy group, e.g., methanesulfonyloxy and butanesulfonyloxy), an arenesulfonyloxy group (preferably a 6- to 12-carbon arenesulfonyloxy group, e.g., benzenesulfonyloxy), an amide group (a 2- to 20-carbon, preferably 2- to 10-carbon amide group, e.g., acetamide, pentane amide, hexane amide, heptane amide, and benzamide), an alkanesulfonamide group (a 1- to 20-carbon, preferably 1- to 10-carbon alkanesulfonamide group, e.g., methanesulfonamide and butanesulfonamide), an arenesulfonamide group (a 6- to 20-carbon, preferably 6- to 15-carbon arenesulfonamide group, e.g., benzenesulfonamide and p-toluenesulfonamide), an alkoxy carbonylamino group (a 1- to 20-carbon, preferably 1- to 10-carbon alkoxy carbonylamino group, e.g., ethoxycarbonylamino), a cycloalkyloxycarbonylamino group (preferably a 4- to 10-carbon cycloalkyloxycarbonylamino group, e.g., cyclohexyloxycarbonylamino), an aryloxycarbonylamino group (a 7- to 20-carbon, preferably a 7- to 15-carbon aryloxycarbonylamino group, e.g., phenoxy carbonylamino), a ureido group (a 1- to 20-carbon, preferably 1- to 10-carbon ureido group, e.g., N-phenylureido), a nitro group, an acyl group (a 1- to 20-, preferably 2- to 10-carbon acyl group, e.g., acetyl and benzoyl), an alkoxy carbonyl group (a 2- to 20-carbon, preferably 2- to 10-carbon alkoxy carbonyl group, methoxycarbonyl, butoxycarbonylmethoxycarbonyl, and isoamyl oxycarbonylmethoxycarbonyl), a cycloalkyloxycarbonyl group (preferably a 4- to 10-carbon cycloalkyloxycarbonyl group, e.g., cyclopropyloxycarbonyl and cyclohexyloxycarbonyl), an aryloxycarbonyl group (a 7- to 21-carbon, preferably 7- to 11-carbon aryloxycarbonyl group, e.g., phenoxy carbonyl), a carbamoyl group (a 1- to 20-carbon, preferably 1- to 10-carbon carbamoyl group, e.g., N-butyl carbamoyl, N,N-diethyl carbamoyl, and N-methyl carbamoyl), a cyano group, an alkylthio group (a 1- to 20-carbon, preferably 1- to 10-carbon alkylthio group, e.g., methylthio, butylthio, and hexylthio), an arylthio group (a 6- to 20-carbon, preferably 6- to 15-carbon arylthio group, e.g., phenylthio and naphthylthio), an alkanesulfonyl group (a 1- to 20-carbon, preferably 1- to 10-carbon alkanesulfonyl group, e.g., methanesulfonyl and butanesulfonyl), an arenesulfonyl group (a 6- to 20-carbon, preferably 6- to 15-carbon arenesulfonyl group, e.g., benzenesulfonyl and p-toluenesulfonyl), an alkoxy sulfonyl group (preferably a 1- to 10-carbon alkoxy sulfonyl group, e.g., methoxysulfonyl and ethoxysulfonyl), a cycloalkyloxysulfonyl group (preferably a 3- to 10-carbon cycloalkyloxysulfonyl group, e.g., cyclopropyloxysulfonyl), an aryloxysulfonyl group (preferably a 6- to 12-carbon aryloxysulfonyl group, e.g., phenoxy sulfonyl and p-methylphenoxy sulfonyl), and a sulfamoyl group (a 1- to 20-carbon, preferably 1- to 10-carbon sulfamoyl group, e.g., N-butyl sulfamoyl and N,N-dimethyl sulfamoyl). Each of the above groups can be either substituted or nonsubstituted. R<sub>91</sub> can further have substituent groups. Preferable substituent groups are those enumerated as R<sub>92</sub>.

R<sub>92</sub> represents an alkyl group, a cycloalkyl group, an aryl group, or a heterocyclic group. Preferable practical examples of these groups are the same as those enumerated in the explanation of R<sub>91</sub>. k represents any number from 0 to 4, and g represents 0 or 1. V represents an oxygen atom, a sulfur atom, or —N(R<sub>93</sub>)— wherein R<sub>93</sub> represents a group having the same meaning as R<sub>92</sub>.

DI is particularly preferably DI-1 or DI-2.

Preferable R<sub>91</sub>, R<sub>92</sub>, and V in DI-1 and DI-2 will be described below.

In DI-1, R<sub>92</sub> is preferably an alkyl group or an aryl group.

Preferable carbon numbers and practical examples of these alkyl and aryl groups are the same as those of the substituent groups enumerated above as R<sub>91</sub>.

R<sub>92</sub> is particularly preferably represented by —CH<sub>2</sub>CO<sub>2</sub>—R or —CH<sub>2</sub>CH<sub>2</sub>CO<sub>2</sub>—R wherein R represents —C<sub>4</sub>H<sub>9</sub>, —C<sub>5</sub>H<sub>11</sub>—n, —C<sub>5</sub>H<sub>11</sub>—i, —CH<sub>2</sub>CH=CHCH<sub>3</sub>, or —CH<sub>2</sub>CH=C(CH<sub>3</sub>)<sub>2</sub>.

In DI-2, V is preferably an oxygen atom or a sulfur atom.

In DI-2, R<sub>91</sub> is preferably an alkylthio group or an arylthio group. R<sub>91</sub> is particularly preferably represented by —SCH<sub>2</sub>CO<sub>2</sub>—R, —SCH<sub>2</sub>CH<sub>2</sub>CO<sub>2</sub>—R, or —SCH(CH<sub>3</sub>)CO<sub>2</sub>—R wherein R has the same meanings as explained above in the preferable examples of R<sub>92</sub>.

Practical examples of preferable development inhibitors are presented below, but the present invention is not limited by these examples.



**15**

-continued

**16**

-continued



45 As described previously, a compound represented by formula (I) is preferably represented by formula (II). Preferable combinations of A and DI in formula (II) will be described below.

50 In a compound represented by formula (II), it is preferable that a group represented by A be formula (Cp-1), (Cp-2), (Cp-6), (Cp-7), (Cp-8), or (Cp-11) and DI be formula (DI-1), (DI-2), or (DI-3). It is more preferable that a group represented by A be formula (Cp-1) or (Cp-8) and DI be formula 55 (DI-1) or (DI-2).

Practical examples of a coupler represented by formula (I) of the present invention are presented below, but the present invention is not limited to these examples.

(1)



(2)



(3)



19

-continued



20

(4)



(5)



(6)

-continued



(7)



(8)



(9)

-continued



(10)



(11)



(12)

-continued

(13)



(14)



(15)



-continued

(16)



(17)



(18)



29

-continued



(19)



(20)



(21)

-continued

(22)



(23)



(24)



-continued

(25)



(26)



(27)



-continued

(28)



(29)



(30)



-continued



(31)



(32)



(33)



(34)

39

-continued

40

(35)



(36)



(37)



-continued

(38)



(39)



(40)



-continued

(41)



(42)



(43)



-continued

(44)



(45)



(46)



-continued

(47)



(48)



Compounds of the present invention can be synthesized in accordance with methods described in Jpn. Pat. Appln. KOKAI Publication Nos. 5-313322 (JP-A-5-313322) and 5-331145.

Practical synthesis examples of compounds of the present invention will be described below. Synthesis example 1 (synthesis of example compound (1))

An example compound (1) was synthesized by the following reaction formula.



35

40

45

60

50

55

65



-continued



Example compound (1)

65

## Synthesis of Intermediate (I-3)

40.0 g of (I-1) and 17.5 g of (I-2) were dissolved in 300 ml of ethyl acetate, and 23 ml of triethylamine were added to the solution. The resultant mixture was stirred at 80° C. for 3 hr. The reaction mixture was cooled with ice, and 200 ml of 1 N hydrochloric acid and 300 ml of hexane were sequentially added. The precipitated crystal was filtered, washed with hexane, and dried to obtain an intermediate (I-3) weighing 18.0 g (yield 37%).

## Synthesis of Intermediate (I-4)

A mixture of 18.0 g of (I-3), 10.0 g of paraformaldehyde, 30 ml of acetic acid, and 100 ml of 1,2-dichloroethane was heated and reacted under reflux for 10 hr. After being cooled to room temperature, the reaction solution was washed with water and dried with anhydrous sodium sulfate. Thereafter, the solvent was distilled off. The residue was refined through a silica gel column chromatography to obtain an intermediate (I-4) weighing 7.0 g (yield 37%). The structure of the resultant intermediate (I-4) compound was checked by <sup>1</sup>H NMR and a mass spectrum.

<sup>1</sup>H NMR (CDCl<sub>3</sub>), δ 0.90 (3H, t), 1.02 (3H, t), 1.1–1.6 (24H, m), 1.93 (4H, m), 4.10 (2H, m), 4.31 (2H, m), 4.70, 4.93 (2H, s in total because of a stereoisomer mixture), 6.05, 6.22 (2H, s in total), 6.98 (1H, d), 7.05 (1H, t), 7.12 (1H, t), 7.38, 7.40 (1H, s in total), 7.62 (1H, t), 7.70 (1H, t), 7.85, 7.92 (1H, d in total), 8.40 (1H, d), 8.53 (1H, d), 8.70 (1H, s), 13.65 (1H, s) MS m/z 743 (M<sup>+</sup>)

## Synthesis Example 2 (synthesis of example compound (18))

An example compound (18) was synthesized by the following reaction formula.



(1H, d), 6.97 (1H, t), 7.08 (1H, t), 7.28 (1H, s), 7.50–7.80 (3H, m), 8.33 (1H, d), 8.45 (1H, br), 8.63 (1H, br), 13.64 (1H, br). MS m/z 603 (M<sup>+</sup>)

## Synthesis of Example Compound (1)

14.4 g of zinc iodide were added to a mixture of 6.5 g of (I-4), 3.4 g of (I-5), and 100 ml of dichloroethane at room

temperature, and the resultant material was reacted for 15 hr. After 50 ml of 1 N hydrochloric acid were added, the organic layer was sequentially washed with water and saturated salt water. The organic layer was dried with anhydrous sodium sulfate, and the solvent was distilled off. The residue was refined through a silica gel column chromatography to obtain an example compound (I) weighing 3.8 g (yield 48%). The melting point was 100 to 102° C. The structure of the resultant example compound (I) was checked by <sup>1</sup>H NMR and a mass spectrum.

<sup>1</sup>H NMR (CDCl<sub>3</sub>), δ 0.90 (3H, t), 1.02 (3H, t), 1.1–1.6 (24H, m), 1.93 (4H, m), 4.10 (2H, m), 4.31 (2H, m), 4.70, 4.93 (2H, s in total because of a stereoisomer mixture), 6.05, 6.22 (2H, s in total), 6.98 (1H, d), 7.05 (1H, t), 7.12 (1H, t), 7.38, 7.40 (1H, s in total), 7.62 (1H, t), 7.70 (1H, t), 7.85, 7.92 (1H, d in total), 8.40 (1H, d), 8.53 (1H, d), 8.70 (1H, s), 13.65 (1H, s) MS m/z 743 (M<sup>+</sup>)

## Synthesis Example 2 (synthesis of example compound (18))

An example compound (18) was synthesized by the following reaction formula.

## Synthesis of Intermediate (II-3)

A mixture of 100 ml of (II-1) and 200 g of (II-2) was stirred under reduced pressure with an aspirator at 130° C. for 8 hr. The reaction mixture was cooled to 60° C., 800 ml of methanol and 40 ml of water were added to the mixture, and the resultant mixture was again heated and dissolved.

After the resultant material was cooled with standing, the precipitated crystal was filtered, washed with methanol, and dried to obtain an intermediate (II-3) weighing 176 g (yield 71%).

Synthesis of Intermediate (II-4)

120 g of (II-3) were dissolved in 600 ml of dichloromethane, and 12.8 ml of sulfonyl chloride were added to the solution at room temperature. After being stirred at room temperature for 1 hr, the reaction solution was sequentially washed with water and saturated salt water. The organic layer was dried with anhydrous sodium sulfate, and the solvent was distilled off. The residue was dissolved in 130 ml of N,N-dimethylacetamide and 70 ml of acetic acid, 60 g of anhydrous potassium acetate were added to the solution, and the resultant material was stirred at 55° C. for 1 hr. After the reaction mixture was cooled with standing, 800 ml of ethyl acetate were added to the mixture, and the resultant material was sequentially washed with water and saturated salt water. The organic layer was dried with anhydrous sodium sulfate, and the solvent was distilled off. The residue was dissolved in 300 ml of methanol, and 90 ml of 30% ammonia water were added under nitrogen stream. The resultant mixture was heated to 40° C. and reacted for 2 hr. The reaction solution was cooled with ice, and 120 ml of 6 N hydrochloric acid were added. The reaction solution was extracted with ethyl acetate and sequentially washed with water and saturated salt water. The organic layer was dried with anhydrous sodium sulfate, and the solvent was distilled off to obtain a coarse product of an intermediate (II-4) weighing 122 g. This product was directly used in the subsequent reaction without being refined.

Synthesis of Intermediate (II-6)

A mixture of 60 g of (II-5), 8.6 g of paraformaldehyde, 42.9 g of (I-5), 30.3 g of anhydrous copper(II) bromide, and 500 ml of 1,2-dichloroethane was stirred at 45° C. for 10 hr. The reaction mixture was cooled to room temperature, and 300 ml of 1 N hydrochloric acid were added. The organic layer was sequentially washed with water and saturated salt water and dried with anhydrous sodium sulfate, and the solvent was distilled off. The residue was refined through a silica gel column chromatography to obtain an intermediate (II-6) weighing 53 g (yield 50%).

Synthesis of Example Compound (18)

26.7 g of (II-4) and 11.1 g of (II-6) were dissolved in 80 ml of N,N-dimethylformamide, and 18.8 g of anhydrous potassium carbonate were added to the solution under nitrogen stream. The resultant mixture was reacted at room temperature for 3 hr, and 600 ml of ethyl acetate and 300 ml of water were added. The organic layer was sequentially washed with an aqueous potassium carbonate solution, 0.5 N hydrochloric acid, water, and saturated salt water, and dried with anhydrous sodium sulfate. The solvent was distilled off, and the residue was refined through a silica gel column chromatography to obtain an example compound (18) weighing 14.7 g (yield 50%). Amorphous. The structure of the resultant example compound (18) was checked by <sup>1</sup>HNMR and a mass spectrum.

<sup>1</sup>HNMR (CDCl<sub>3</sub>), 80.95 (3H, t), 1.00 (3H, t), 1.1–1.5 (30H, m), 1.92 (2H, m), 2.90 (2H, m), 4.30 (2H, t), 4.80 (2H, m), 5.09 (1H, t), 6.02 (2H, m), 6.52, 6.63 (1H, s in total because of a stereoisomer mixture), 7.25–7.77 (8H, m), 8.0–8.2 (3H, m), 8.57, 8.70 (1H, s in total), 8.83, 9.15 (1H, s in total) MS m/z 1034 (M<sup>+</sup>+1)

A compound represented by formula (I) of the present invention is used in a light-sensitive material to improve the color reproduction by giving a satisfactory interlayer effect to a layer or improve the sharpness. The addition amount is

1×10<sup>-6</sup> to 1×10<sup>-2</sup> mol, preferably 5×10<sup>-5</sup> to 1×10<sup>-3</sup> mol per 1 m<sup>2</sup> of a light-sensitive material.

A compound represented by formula (I) can be used in any of blue-sensitive emulsion layers, green-sensitive emulsion layers, red-sensitive emulsion layers, and non-light-sensitive layers (e.g., interlayers, protective layers, anti-halation layers, and white pigment layers). The compound is preferably used in an underlying layer (formed close to a support) of layers constituting a light-sensitive material. The compound is particularly preferable in development when the color development time of the present invention is shortened.

As a compound represented by formula (I), the same compound can be used in a plurality of layers, different compounds can be used in the same layer, or different compounds can be used in different layers in accordance with the intended use. Furthermore, these compounds can be used together with well-known DIR compounds (e.g., DIR compounds described in R. D. No. 307105).

A compound represented by formula (I) of the present invention is characterized by X<sub>1</sub> in formula (I) with respect to practical compounds described in Jpn. Pat. Appln. KOKAI Publication No. 5-31332 described previously.

Practical compounds equal to X<sub>1</sub> in formula (I) of the present invention are described in Jpn. Pat. Appln. KOKAI Publication No. 7-133259 (JP-A-7-133259). However, these compounds are different from the compounds of the present invention in that a portion corresponding to DI is limited to an azole development inhibitor. Additionally, Jpn. Pat. Appln. KOKAI Publication No. 7-133259 relates to methods of compound synthesis and does not refer to effects on photographic properties at all.

The present invention well achieved the object of the present invention by specifying X<sub>1</sub> in formula (I) and combining mercaptoazole development inhibitors as DI.

In the light-sensitive material of the present invention, at least one light-sensitive layer need only be formed on a support. A typical example is a silver halide photographic light-sensitive material having, on its support, at least one light-sensitive layer constituted by a plurality of silver halide emulsion layers which are sensitive to essentially the same color but have different sensitivities. This light-sensitive layer is a unit sensitive layer which is sensitive to one of blue light, green light, and red light. In a multilayered silver halide color photographic light-sensitive material, such unit light-sensitive layers are generally arranged in the order of red-, green-, and blue-sensitive layers from a support. However, according to the intended use, this arrangement order may be reversed, or light-sensitive layers sensitive to the same color may sandwich another light-sensitive layer sensitive to a different color. Non-light-sensitive layers can be formed between the silver halide light-sensitive layers and as the uppermost layer and the lowermost layer. These non-light-sensitive layers can contain, e.g., couplers, DIR compounds, and color amalgamation preventives to be described later. As a plurality of silver halide emulsion layers constituting each unit light-sensitive layer, as described in West German Patent No. 1,121,470 or British Patent No. 923,045, high- and low-speed emulsion layers are preferably arranged such that the sensitivity is sequentially decreased toward a support. In addition, as described in Jpn. Pat. Appln. KOKAI Publication Nos. 57-112751, 62-200350, 62-206541, and 62-206543, layers may be arranged such that a low-speed emulsion layer is formed farther from a support and a high-speed layer is formed close to the support.

More specifically, layers may be arranged from the farthest side from a support in the order of low-speed blue-

sensitive layer (BL)/high-speed blue-sensitive layer (BH)/high-speed green-sensitive layer (GH)/low-speed green-sensitive layer (GL)/high-speed red-sensitive layer (RH)/low-speed red-sensitive layer (RL), the order of BH/BL/GL/GH/RH/RL, or the order of BH/BL/GH/GL/RL/RH.

In addition, as described in Jpn. Pat. Appln. KOKOKU Publication No. 55-34932, layers may be arranged from the farthest side from a support in the order of blue-sensitive layer/GH/RH/GL/RL. Furthermore, as described in Jpn. Pat. Appln. KOKAI Publication Nos. 56-25738 and 62-63936, layers may be arranged from the farthest side from a support in the order of blue-sensitive layer/GL/RL/GH/RH.

As described in Jpn. Pat. Appln. KOKOKU Publication No. 49-15495, three layers may be arranged such that a silver halide emulsion layer having the highest sensitivity is arranged as an upper layer, a silver halide emulsion layer having sensitivity lower than that of the upper layer is arranged as an interlayer, and a silver halide emulsion layer having sensitivity lower than that of the interlayer is arranged as a lower layer, i.e., three layers having different sensitivities may be arranged such that the sensitivity is sequentially decreased toward the support. When a layer structure is constituted by three layers having different sensitivities, these layers may be arranged in the order of medium-speed emulsion layer/high-speed emulsion layer/low-speed emulsion layer from the farthest side from a support in a layer sensitive to one color as described in Jpn. Pat. Appln. KOKAI Publication No. 59-202464.

In addition, the order of high-speed emulsion layer/low-speed emulsion layer/medium-speed emulsion layer or low-speed emulsion layer/medium-speed emulsion layer/high-speed emulsion layer may be adopted. Furthermore, the arrangement can be changed as described above even when four or more layers are formed.

In order to improve the color reproduction, a donor layer (CL) with an interlayer effect, which is described in U.S. Pat. No. 4,663,271, 4,705,744, or 4,707,436, or Jpn. Pat. Appln. KOKAI Publication No. 62-160448 or 63-89580 and different from the main light-sensitive layers BL, GL, and RL in spectral sensitivity distribution, is preferably formed adjacent to or close to the main light-sensitive layers.

A preferable silver halide used in the present invention is silver iodobromide, silver iodochloride, or silver iodochlorobromide containing about 1 mol % to about 30 mol % of silver iodide. A particularly preferable silver halide is silver iodobromide or silver iodochlorobromide containing about 2 mol % to about 10 mol % of silver iodide.

Silver halide grains contained in the photographic emulsion may have regular crystals such as cubic, octahedral, or tetradecahedral crystals, irregular crystals such as spherical or tabular crystals, crystals having crystal defects such as twinned crystal faces, or composite shapes thereof.

A silver halide can consist of fine grains having a grain size of about 0.2  $\mu\text{m}$  or less or large grains having a projected area diameter of about 10  $\mu\text{m}$ , and an emulsion may be either a polydisperse or monodisperse emulsion.

A silver halide photographic emulsion which can be used in the present invention can be prepared by methods described in, e.g., "I. Emulsion preparation and types," Research Disclosure (RD) No. 17643 (December, 1978), pp. 22 and 23, RD No. 18716 (November, 1979), page 648, and RD No. 307105 (November, 1989), pp. 863 to 865; P. Glafkides, "Chimie et Physique Photographique", Paul Montel, 1967; G. F. Duffin, "Photographic Emulsion Chemistry", Focal Press, 1966; and V. L. Zelikman et al., "Making and Coating Photographic Emulsion", Focal Press, 1964.

Monodisperse emulsions described in, for example, U.S. Pat. Nos. 3,574,628 and 3,655,394 and British Patent No. 1,413,748 are also preferable.

Also, tabular grains having an aspect ratio of about 3 to 50 can be used in the present invention. Tabular grains can be easily prepared by methods described in, e.g., Gutoff, "Photographic Science and Engineering", Vol. 14, pp. 248 to 257 (1970); U.S. Pat. Nos. 4,434,226, 4,414,310, 4,433,048, and 4,439,520, and British Patent No. 2,112,157.

10 A crystal structure can be uniform, can have different halogen compositions in the interior and the surface layer thereof, or can be a layered structure. Alternatively, a silver halide having a different composition can be bonded by an epitaxial junction, or a compound except for a silver halide such as silver rhodanide or zinc oxide can be bonded. A mixture of grains having various types of crystal shapes can also be used.

The above emulsion can be any of a surface latent image type emulsion which mainly forms a latent image on the 20 surface of a grain, an internal latent image type emulsion which forms a latent image in the interior of a grain, and an emulsion of another type which has latent images on the surface and in the interior of a grain. However, the emulsion must be a negative type emulsion. The internal latent image 25 type emulsion can be a core/shell internal latent image type emulsion described in Jpn. Pat. Appln. KOKAI Publication No. 63-264740. A method of preparing this core/shell internal latent image type emulsion is described in Jpn. Pat. Appln. KOKAI Publication No. 59-133542. Although the 30 thickness of a shell of this emulsion depends on, e.g., development conditions, it is preferably 3 to 40 nm, and most preferably 5 to 20 nm.

A silver halide emulsion layer is normally subjected to physical ripening, chemical ripening, and spectral sensitization steps before it is used. Additives for use in these steps are described in RD Nos. 17643, 18716, and 307105, and they are summarized in a table presented later.

In the light-sensitive material of the present invention, it is possible to simultaneously use, in a single layer, two or 40 more types of emulsions different in at least one of the characteristics of a light-sensitive silver halide emulsion, i.e., the grain size, grain size distribution, halogen composition, grain shape, and sensitivity.

It is also possible to preferably use surface-fogged silver 45 halide grains described in U.S. Pat. No. 4,082,553, internally fogged silver halide grains described in U.S. Pat. No. 4,626,498 and Jpn. Pat. Appln. KOKAI Publication No. 59-214852, and colloidal silver, in light-sensitive silver halide emulsion layers and/or essentially non-light-sensitive 50 hydrophilic colloid layers. The internally fogged or surface-fogged silver halide grain means a silver halide grain which can be developed uniformly (non-imagewise) regardless of whether the location is a non-exposed portion or an exposed portion of the light-sensitive material. Methods of preparing the internally fogged or surface-fogged silver halide grain are described in U.S. Pat. No. 4,626,498 and Jpn. Pat. Appln. KOKAI Publication No. 59-214852. A silver halide which forms the core of an internally fogged core/shell type silver halide grain can have a different halogen composition. As 55 the internally fogged or surface-fogged silver halide, any of silver chloride, silver chlorobromide, silver iodobromide, and silver iodochlorobromide can be used. The grain size of these fogged silver halide grains is preferably 0.01 to 0.75  $\mu\text{m}$ , and particularly preferably 0.05 to 0.6  $\mu\text{m}$ . The grains can also be regular grains, and the emulsion can be a polydisperse emulsion. However, the emulsion is preferably 60 a monodisperse emulsion (in which at least 95% of the

weight or number of grains of silver halide grains have grain sizes within  $\pm 40\%$  of an average grain size).

In the present invention, it is preferable to use a non-light-sensitive fine grain silver halide. The non-light-sensitive fine grain silver halide preferably consists of fine silver halide grains which are not exposed during imagewise exposure for obtaining a dye image and are not essentially developed during development. These fine silver halide grains are preferably not fogged in advance. The fine grain silver halide contains 0 to 100 mol % of silver bromide and can also contain silver chloride and/or silver iodide if necessary. The fine grain silver halide preferably contains 0.5 to 10 mol % of silver iodide. The average grain size (the average value of equivalent circle diameters of projected areas) of the fine grain silver halide is preferably 0.01 to 0.5  $\mu\text{m}$ , and more preferably 0.02 to 0.2  $\mu\text{m}$ .

The fine grain silver halide can be prepared following the same procedures as for a common light-sensitive silver halide. In this case, the surface of each silver halide grain need not be optically sensitized nor spectrally sensitized. However, before the silver halide grains are added to a coating solution, it is preferable to add a well-known stabilizer such as a triazole-based compound, an azaindene-based compound, a benzothiazolium-based compound, a mercapto-based compound, or a zinc compound. Colloidal silver can be added to this fine grain silver halide-containing layer.

The silver coating amount of the light-sensitive material of the present invention is preferably 0.1 g/m<sup>2</sup> to 6.0 g/m<sup>2</sup>, and most preferably 0.2 g/m<sup>2</sup> to 4.5 g/m<sup>2</sup>.

Photographic additives usable in the present invention are also described in RDs, and the corresponding portions are summarized in the following table.

| Additives                                               | RD17643       | RD18716                                          |
|---------------------------------------------------------|---------------|--------------------------------------------------|
| 1. Chemical sensitizers                                 | page 23       | page 648, right column                           |
| 2. Sensitivity increasing agents                        |               | page 648, right column                           |
| 3. Spectral sensitizers, super sensitizers              | pages 23–24   | page 648, right column to page 649, right column |
| 4. Brighteners                                          | page 24       | page 647, right column                           |
| 5. Light absorbent, filter dye, ultra-violet absorbents | pages 25–26   | page 649, right column to page 650, left column  |
| 6. Binder                                               | page 26       | page 651, left column                            |
| 7. Plasticizers, lubricants                             | page 27       | page 650, right column                           |
| 8. Coating aids, surface active agents                  | pages 26–27   | page 650, right column                           |
| 9. Antistatic agents                                    | page 27       | page 650, right column                           |
| 10. Matting agent                                       |               |                                                  |
| Additives                                               | RD307105      |                                                  |
| 1. Chemical sensitizers                                 | page 866      |                                                  |
| 2. Sensitivity increasing agents                        |               |                                                  |
| 3. Spectral sensitizers, super sensitizers              | pages 866–868 |                                                  |
| 4. Brighteners                                          | page 868      |                                                  |
| 5. Light absorbent, filter dye, ultra-violet absorbents | page 873      |                                                  |
| 6. Binder                                               | pages 873–874 |                                                  |

-continued

|     | Additives                           | RD17643       | RD18716 |
|-----|-------------------------------------|---------------|---------|
| 7.  | Plasticizers, lubricants            | page 876      |         |
| 8.  | Coating aids, surface active agents | pages 875–876 |         |
| 9.  | Antistatic agents                   | pages 876–877 |         |
| 10. | Matting agent                       | pages 878–879 |         |

10 Various dye forming couplers can be used in the light-sensitive material of the present invention, and the following couplers are particularly preferable.

Yellow couplers: couplers represented by formulas (I) and (II) in EP 502,424A; couplers (particularly Y-28 on page 18) represented by formulas (1) and (2) in EP 513,496A; a coupler represented by formula (I) in claim 1 of EP 568, 037A; a coupler represented by Formula (I) in column 1, lines 45 to 55, in U.S. Pat. No. 5,066,576; a coupler represented by formula (I) in paragraph 0008 of Jpn. Pat. Appln. KOKAI Publication No. 4-274425; couplers (particularly D-35 on page 18) described in claim 1 on page 40 in EP 498,381A1; couplers (particularly Y-1 (page 17) and Y-54 (page 41)) represented by formula (Y) on page 4 25 in EP 447,969A1; and couplers (particularly II-17, II-19 (column 17), and II-24 (column 19)) represented by formulas (II) to (IV) in column 7, lines 36 to 58, in U.S. Pat. No. 4,476,219.

Magenta couplers: Jpn. Pat. Appln. KOKAI Publication 30 No. 3-39737 (L-57 (page 11, lower right column), L-68 (page 12, lower right column), and L-77 (page 13, lower right column); (A-4)-63 (page 134), and (A-4)-73 and (A-4)-75 (page 139) in EP 456,257; M-4 and M-6 (page 26), and M-7 (page 27) in EP 486,965; M-45 (page 19) in EP 35 571,959A; (M-1) (page 6) in Jpn. Pat. Appln. KOKAI Publication No. 5-204106; and M-22 in paragraph 0237 of Jpn. Pat. Appln. KOKAI Publication No. 4-362631.

Cyan couplers: CX-1, CX-3, CX-4, CX-5, CX-11, CX-12, CX-14, and CX-15 (pages 14 to 16) in Jpn. Pat. Appln. 40 KOKAI Publication No. 4-204843; C-7 and C-10 (page 35), C-34 and C-35 (page 37), and (I-1) and (I-17) (pages 42 and 43) in Jpn. Pat. Appln. KOKAI Publication No. 4-43345; and couplers represented by formulas (Ia) and (Ib) in claim 1 of Jpn. Pat. Appln. KOKAI Publication No. 6-67385.

45 Polymer couplers: P-1 and P-5 (page 11) in Jpn. Pat. Appln. KOKAI Publication No. 2-44345.

Couplers for forming a colored dye with a proper diffusibility are preferably those described in U.S. Pat. No. 4,366,237, GB 2,125,570, EP 96,873B, and DE 3,234,533.

50 Couplers for correcting unnecessary absorption of a colored dye are preferably yellow colored cyan couplers (particularly YC-86 on page 84) represented by formulas (CI), (CII), (CIII), and (CIV) described on page 5 in EP 456,257A1; yellow colored magenta couplers ExM-7 (page 202), EX-1 (page 249), and EX-7 (page 251) in EP 456, 257A1; magenta colored cyan couplers CC-9 (column 8) and CC-13 (column 10) described in U.S. Pat. No. 4,833, 069; (2) (column 8) in U.S. Pat. No. 4,837,136; and colorless masking couplers (particularly example compounds on 60 pages 36 to 45) represented by formula (A) in claim 1 of WO 92/11575.

65 Examples of a compound (including a coupler) which reacts with a developing agent oxidized form and releases a photographically useful compound residue are as follows. Development inhibitor release compounds: compounds (particularly T-101 (page 30), T-104 (page 31), T-113 (page 36), T-131 (page 45), T-144 (page 51), and T-158 (page 58))

represented by formulas (I), (II), (III), and (IV) described on page 11 in EP 378,236A1, compounds (particularly D-49 (page 51) represented by formula (I) described on page 7 in EP 436,938A2, compounds (particularly (23) (page 11) represented by formula (1) in EP 568,037A, and compounds (particularly I-(1) on page 29) represented by formulas (I), (II), and (III) described on pages 5 and 6 in EP 440,195A2; bleaching accelerator release compounds: compounds (particularly (60) and (61) on page 61) represented by formulas (I) and (I') on page 5 of EP 310,125A2, and compounds (particularly (7) (page 7)) represented by formula (I) in claim 1 of Jpn. Pat. Appln. KOKAI Publication No. 6-59411; ligand release compound: compounds (particularly compounds in column 12, lines 21 to 41) represented by LIG-X described in claim 1 of U.S. Pat. No. 4,555,478; leuco dye release compounds: compounds 1 to 6 in columns 3 to 8 of U.S. Pat. No. 4,749,641; fluorescent dye release compounds: compounds (particularly compounds 1 to 11 in columns 7 to 10) represented by COUP-DYE in claim 1 of U.S. Pat. No. 4,774,181; development accelerator or fogging agent release compounds: compounds (particularly (I-22) in column 25) represented by formulas (1), (2), and (3) in column 3 of U.S. Pat. No. 4,656,123, and ExZK-2 on page 75, lines 36 to 38, in EP 450,637A2; compounds which release a group which does not function as a dye unless it splits off: compounds (particularly Y-1 to Y-19 in columns 25 to 36) represented by formula (I) in claim 1 of U.S. Pat. No. 4,857,447.

Preferable examples of additives other than couplers are as follows.

Dispersants of an oil-soluble organic compound: P-3, P-5, P-16, P-19, P-25, P-30, P-42, P-49, P-54, P-55, P-66, P-81, P-85, P-86, and P-93 (pages 140 to 144) in Jpn. Pat. Appln. KOKAI Publication No. 62-215272; impregnating latexes of an oil-soluble organic compound: latexes described in U.S. Pat. No. 4,199,363; developing agent oxidized form scavengers: compounds (particularly I-(1), I-(2), I-(6), and I-(12) (columns 4 and 5)) represented by formula (I) in column 2, lines 54 to 62, in U.S. Pat. No. 4,978,606, and formulas (particularly compound 1 (column 3)) in column 2, lines 5 to 10, in U.S. Pat. No. 4,923,787; stain inhibitors: formulas (I) to (III) on page 4, lines 30 to 33, particularly I-47, I-72, III-1, and III-27 (pages 24 to 48) in EP 298321A; brown inhibitors: A-6, A-7, A-20, A-21, A-23, A-24, A-25, A-26, A-30, A-37, A-40, A-42, A-48, A-63, A-90, A-92, A-94, and A-164 (pages 69 to 118) in EP 298321A, II-III-23, particularly III-10, in columns 25 to 38 of U.S. Pat. No. 5,122,444, I-1 to III-4, particularly II-2, on pages 8 to 12 in EP 471347A, and A-1 to A-48, particularly A-39 and A-42, in columns 32 to 40 of U.S. Pat. No. 5,139,931; materials which reduce the use amount of a color enhancer or a color amalgamation preventives: I-1 to II-15, particularly I-46, on pages 5 to 24 in EP 411324A; formalin scavengers: SCV-1 to SCV-28, particularly SCV-8, on pages 24 to 29 in EP 477932A; film hardeners: H-1, H-4, H-6, H-8, and H-14 on page 17 in Jpn. Pat. Appln. KOKAI Publication No. 1-214845, compounds (H-1 to H-54) represented by formulas (VII) to (XII) in columns 13 to 23 of U.S. Pat. No. 4,618,573, compounds (H-1 to H-76), particularly H-14, represented by formula (6) on page 8, lower right column, in Jpn. Pat. Appln. KOKAI Publication No. 2-214852, and compounds described in claim 1 of U.S. Pat. No. 3,325,287;

development inhibitor precursors: P-24, P-37, and P-39 (pages 6 and 7) in Jpn. Pat. Appln. KOKAI Publication No. 62-168139; compounds described in claim 1, particularly 28 and 29 in column 7, of U.S. Pat. No. 5,019,492; antiseptic agents and mildewproofing agents: I-1 to III-43, particularly

II-1, II-9, II-10, II-18, and III-25, in columns 3 to 15 of U.S. Pat. No. 4,923,790; stabilizers and antifoggants: I-1 to (14), particularly I-1, I-60, (2), and (13), in columns 6 to 16 of U.S. Pat. No. 4,923,793, and compounds 1 to 65, particularly compound 36, in columns 25 to 32 of U.S. Pat. No. 4,952,483; chemical sensitizers: triphenylphosphine selenide and compound 50 in Jpn. Pat. Appln. KOKAI Publication No. 5-40324; dyes: a-1 to b-20, particularly a-1, a-12, a-18, a-27, a-35, a-36, and b-5, on pages 15 to 18 and V-1 to V-23, particularly V-1, on pages 27 to 29 in Jpn. Pat. Appln. KOKAI Publication No. 3-156450, F-I-1 to F-II-43, particularly F-I-11 and F-II-8, on pages 33 to 55 in EP 445627A, III-1 to III-36, particularly III-1 and III-3, on pages 17 to 28 in EP 457153A, fine crystal dispersions of Dye-1 to Dye-124 on pages 8 to 26 in WO 88/04794, compounds 1 to 22, particularly compound 1, on pages 6 to 11 in EP 319999A, compounds D-1 to D-87 (pages 3 to 28) represented by formulas (1) to (3) in EP 519306A, compounds 1 to 22 (columns 3 to 10) represented by formula (I) in U.S. Pat. No. 4,268,622, and compounds (1) to (31) (columns 2 to 9) represented by formula (I) in U.S. Pat. No. 4,923,788; UV absorbents: compounds (18b) to (18r) and 101 to 427 (pages 6 to 9) represented by formula (1) in Jpn. Pat. Appln. KOKAI Publication No. 46-3335, compounds (3) to (66) (pages 10 to 44) and compounds HBT-1 to HBT-10 (page 14) represented by formula (III) in EP 520938A, and compounds (1) to (31) (columns 2 to 9) represented by formula (1) in EP 521823A.

The present invention can be applied to various color 30 light-sensitive materials such as a color negative film for a general purpose or a movie, a color reversal film for a slide or a television, color paper, a color positive film, and color reversal paper. The present invention is also suited to film units with lens described in Jpn. Pat. Appln. KOKOKU Publication No. 2-32615 and Jpn. Utility Model Appln. KOKOKU Publication No. 3-39784.

A support which can be suitably used in the present invention is described in, e.g., RD. No. 17643, page 28, RD. No. 18716, from the right column, page 647 to the left 40 column, page 648, and RD. No. 307105, page 879.

In the light-sensitive material of the present invention, the total film thickness of all hydrophilic colloid layers on the side having emulsion layers is preferably 28  $\mu\text{m}$  or less, more preferably 23  $\mu\text{m}$  or less, particularly preferably 18  $\mu\text{m}$  or less, and most preferably 16  $\mu\text{m}$  or less. A film swell speed  $T_{1/2}$  is preferably 30 sec or less, and more preferably, 20 sec or less.  $T_{1/2}$  is defined as a time which the film thickness requires to reach  $\frac{1}{2}$  of a saturation film thickness which is 45 90% of a maximum swell film thickness reached when processing is performed by using a color developer at 30°C. for 3 min and 15 sec. The film thickness means the thickness of a film measured under moisture conditioning at a temperature of 25°C. and a relative humidity of 55% (two days).  $T_{1/2}$  can be measured by using a swell meter described 50 in Photogr. Sci. Eng., A. Green et al., Vol. 19, No. 2, pp. 124 to 129.  $T_{1/2}$  can be adjusted by adding a film hardening agent to gelatin as a binder or changing aging conditions after coating. The swell ratio is preferably 150 to 400%. The swell ratio can be calculated from the maximum swell film thickness under the conditions mentioned above by using 55 (maximum swell film thickness—film thickness)/film thickness.

In the light-sensitive material of the present invention, hydrophilic colloid layers (called back layers) having a total dried film thickness of 2 to 20  $\mu\text{m}$  are preferably formed on the side opposite to the side having emulsion layers. The back layers preferably contain, e.g., the light absorbent, the

filter dye, the ultraviolet absorbent, the antistatic agent, the film hardener, the binder, the plasticizer, the lubricant, the coating aid, and the surfactant described above. The lubrication ratio of the back layers is preferably 150 to 500%.

The light-sensitive material of the present invention can be developed by conventional methods described in RD. No. 17643, pages 28 and 29, RD. No. 18716, page 651, left column to right column, and RD. No. 307105, pages 880 and 881.

Processing solutions used for color negative films in the present invention will be described below.

Compounds described in Jpn. Pat. Appln. KOKAI Publication No. 4-121739, page 9, upper right column, line 1 to page 11, lower left column, line 4 can be used in color developers used in the present invention. In performing rapid processing, color developing agents are preferably 2-methyl-4-(N-ethyl-N-(2-hydroxyethyl)amino)aniline, 2-methyl-4-(N-ethyl-N-(3-hydroxypropyl)amino)aniline, and 2-methyl-4-(N-ethyl-N-(4-hydroxybutyl)amino)aniline.

The use amount of these color developing agents is preferably 0.01 to 0.08 mol, more preferably 0.015 to 0.06 mol, and most preferably 0.02 to 0.05 mol per 1 l of a color developer. A replenishment solution of the color developer is made contain a color developing agent whose concentration is preferably 1.1 to 3 times, and particularly preferably 1.3 to 2.5 times the above concentration.

Hydroxylamine can be extensively used as a preservative of the color developer. When a higher preservability is necessary, hydroxylamine derivatives having substituent groups such as an alkyl group, a hydroxyalkyl group, a sulfoalkyl group, and a carboxyalkyl group are preferable. Practical preferable examples are N,N-di(sulfoethyl)hydroxylamine, monomethylhydroxylamine, dimethylhydroxylamine, monoethylhydroxylamine, diethylhydroxylamine, N,N-di(carboxyethyl)hydroxylamine. Of these hydroxylamine derivatives, N,N-di(sulfoethyl)hydroxylamine is particularly preferable. Although these hydroxylamine derivatives can be used together with hydroxylamine, it is preferable that any of these derivatives be used in combination with one or more different types of derivatives instead of hydroxylamine.

The use amount of the preservative is preferably 0.02 to 0.2 mol, more preferably 0.03 to 0.15 mol, and most preferably 0.04 to 0.1 mol per 1 l. Also, as in the case of the color developing agent, a replenishment solution is preferably made contain a preservative whose concentration is 1.1 to 3 times the concentration of a mother solution (processing tank solution).

In the color developer, sulfite is used as a tar preventing agent for an oxidized form of the color developing agent. The use amount of sulfite is preferably 0.01 to 0.05 mol, and particularly preferably 0.02 to 0.04 mol per 1 l. In a replenishment solution, the concentration of sulfite is preferably 1.1 to 3 times the above value.

The pH of the color developer is preferably 9.8 to 11.0, and particularly preferably 10.0 to 10.5. In a replenishment solution, the pH is preferably higher by 0.1 to 1.0 than these values. To stably maintain such pH, well-known buffering agents such as carbonate, phosphate, sulfosalicylate, and borate are used.

The quantity of replenisher of the color developer is preferably 80 to 1300 ml per 1 m<sup>2</sup> of a light-sensitive material. To reduce environmental contamination, however, the quantity of replenisher is preferably as low as possible. More specifically, the quantity of replenisher is preferably 80 to 600 ml, and more preferably 80 to 400 ml.

A bromide ion concentration in the color developer is usually 0.01 to 0.06 mol per l. However, to suppress the fog

and improve the discrimination and graininess while holding the sensitivity, the bromide ion concentration is preferably set at 0.015 to 0.03 mol per l. To set the bromide ion concentration in this range, it is only necessary to add bromide ion calculated by the following equation to the replenishment solution. If C is negative, it is preferable that no bromide ion be contained in the replenishment solution.

$$C = A - W/V$$

10 C: a bromide ion concentration (mol/l) in a color developer replenishment solution.

A: a target bromide ion concentration (mol/l) in a color developer.

W: an amount (mol) of bromide ion dissolves from a light-sensitive material into a color developer when 1 m<sup>2</sup> of a light-sensitive material is color-developed.

V: a quantity of replenisher (l) of a color developer replenishment solution per 1 m<sup>2</sup> of a light-sensitive material.

To increase the sensitive when the quantity of replenisher is decreased or a high bromide ion concentration is set, it is also preferable to use development accelerators such as pyrazolidones represented by 1-phenyl-3-pyrazolidone and 1-phenyl-2-methyl-2-hydroxymethyl-3-pyrazolidone and a thioether compound represented by 3,6-dithia-1,8-octanediol.

25 As the developing agents used in the present invention, hydrazine type developing agents can also be used in addition to the above-mentioned developing agents. More specifically, hydrazine type compounds described in Japanese Patent Application Nos. 7-63572, 7-343190, 7-334192, 7-334197, and 7-344396 can be preferably used.

30 As a method of development using these agents, it is possible to use wet methods such as a method by which development is performed by using a developer containing a conventional alkali agent and the developing agent and a method by which the developing agent is contained in a light-sensitive material and development is performed by using an activator solution, e.g., an alkali solution, containing no developing agent. In addition to these wet method, a heat development method can also be used.

35 When the activator method is used, it is also preferable to use a development method in which image amplification processing (intensification processing) using hydrogen peroxide is performed by reducing the silver coating amount in a light-sensitive material. More specifically, image formation methods using an activator solution containing hydrogen peroxide described in Japanese Patent Application Nos. 7-63587 and 7-334202 are preferably used.

40 Compounds and processing conditions described in Jpn. Pat. Appln. KOKAI Publication No. 4-125558, page 4, lower left column, line 16 to page 7, lower left column, line 6 can be applied to the processing solution with bleaching capacity according to the present invention.

45 The bleaching agent preferably has an oxidation reduction potential of 150 mV or more, and practical preferable examples are described in Jpn. Pat. Appln. KOKAI Publication Nos. 5-72694 and 5-173312. In particular, 1,3-diaminopropane tetraacetic acid and ferric complex salt of a compound of Example 1 on page 7 of Jpn. Pat. Appln. KOKAI Publication No. 5-173312 are preferable.

50 To improve the biodegradability of the bleaching agent, it is preferable to use any of compound ferric complex salts described in Jpn. Pat. Appln. KOKAI Publication Nos. 4-251845 and 4-268552, European Patent Nos. 588,289 and 591,934, and Jpn. Pat. Appln. KOKAI Publication No.

6-208213 as the bleaching agent. The concentration of these bleaching agents is preferably 0.05 to 0.3 mol per 1 l of the solution with bleaching capacity. To reduce the amount exhausted to the environment, the concentration is preferably designed to be 0.1 to 0.15 mol. If the solution with bleaching capacity is a bleaching solution, preferably 0.2 to 1 mol, and more preferably 0.3 to 0.8 mol of a bromide is contained per l.

A replenishment solution of the solution with bleaching capacity is basically made contain components at concentrations calculated by the following equation. This keeps the concentration in a mother solution constant.

$$C_R = C_T \times (V_1 + V_2) / V_1 + C_p$$

$C_R$ : a concentration of a component in a replenishment solution.

$C_T$ : a concentration of a component in a mother solution (processing tank solution).

$C_p$ : a concentration of a component consumed during processing.

$V_1$ : a quantity of replenisher (ml) of a replenishment solution with bleaching capacity per 1 m<sup>2</sup> of a light-sensitive material.

$V_2$ : an amount (ml) carried over from a preceding bath by m<sup>2</sup> of a light-sensitive material.

In addition, the bleaching solution is preferably made contain a pH buffering agent, particularly dicarboxylic acid having little odor such as succinic acid, maleic acid, malonic acid, glutaric acid, or adipic acid. It is also preferable to use well-known bleaching accelerators described in Jpn. Pat. Appln. KOKAI Publication No. 53-95630, RD No. 17129, and U.S. Pat. No. 3,893,858.

It is preferable to replenish preferably 50 to 1000 ml, more preferably 80 to 500 ml, and most preferably 100 to 300 ml of a bleaching replenishment solution to the bleaching solution per 1 m<sup>2</sup> of a light-sensitive material. Furthermore, aeration is preferably performed for the bleaching solution.

Compounds and processing conditions described in Jpn. Pat. Appln. KOKAI Publication No. 4-125558, page 7, lower left column, line 10 to page 8, lower right column, line 19 can be applied to the processing solution with fixing capacity.

To improve the fixing speed and the preservability, compounds represented by formulas (I) and (II) in Jpn. Pat. Appln. KOKAI Publication No. 6-301169 are preferably added singly or jointly to the processing solution with fixing capacity. Also, the use of sulfonic acid such as p-toluenesulfonate described in Jpn. Pat. Appln. KOKAI Publication No. 1-224762 is preferable to improve the preservability.

In the solution with bleaching capacity and the solution with fixing capacity, the use of ammonium as cation is preferable to improve the desilvering characteristics. However, to reduce environmental contamination, ammonium is preferably reduced or not used.

In the bleaching, bleach-fix, and fixing steps, it is particularly preferable to perform jet stirring described in Jpn. Pat. Appln. KOKAI Publication No. 1-309059.

The quantity of replenisher of a replenishment solution in the bleach-fix or fixing step is 100 to 1000 ml, preferably 150 to 700 ml, and particularly preferably 200 to 600 ml per 1 m<sup>2</sup> of a light-sensitive material.

In the bleach-fix or fixing step, various silver recovery devices are preferably arranged as in-line or off-line devices to recover silver. When the in-line arrangement is used,

processing can be performed while the silver concentration in a solution is decreased. As a consequence, the quantity of replenisher can be decreased. It is also preferable to recover silver by the off-line arrangement and reuse the residual solution as a replenishment solution.

The bleach-fix step or the fixing step can be constituted by a plurality of processing tanks, and these tanks are preferably cascaded to form a multistage counterflow system. To balance the size of a developing solution, a two-tank cascaded configuration is generally efficient. The processing time ratio of the preceding tank to the succeeding tank is preferably 0.5:1 to 1:0.5, and most preferably 0.8:1 to 1:0.8.

In the bleach-fix bath and the fixing solution, a free chelating agent which has not become a metal complex is preferably made exist to improve the preservability. As these chelating agents, the use of biodegradable chelating agents described above in connection with the bleaching solution is preferable.

The contents described in Jpn. Pat. Appln. KOKAI Publication No. 4-125558, page 12, lower right column, line 6 to page 13, lower right column, line 16 can be preferably applied to the washing and stabilization steps. To preserve the work environment, it is preferable to use azolylmethylenamines described in European Patent Nos. 504,609 and 519,190 or N-methylolazoles described in Jpn. Pat. Appln. KOKAI Publication No. 4-362943, instead of formaldehyde, in the stabilizer, or to prepare a solution of a surfactant not containing an image stabilizing agent such as formaldehyde by making a magenta coupler divalent.

To reduce adhesion of dust to a magnetic recording layer applied on a light-sensitive material, a stabilizer described in Jpn. Pat. Appln. KOKAI Publication No. 6-289559 can be preferably used.

The quantity of replenisher of the washing solution and the stabilizer is preferably 80 to 1000 ml, more preferably 100 to 500 ml, and most preferably 150 to 300 ml per 1 m<sup>2</sup> of a light-sensitive material, in order to secure the washing or stabilizing function and reduce the waste solutions for environmental preservation. To prevent the propagation of bacteria and mildew in the processing performed with this quantity of replenisher, it is preferable to use well-known mildewproofing agents such as thiabendazole, 1,2-benzisothiazoline-3-one, 5-chloro-2-methylisothiazoline-3-one, antibiotics such as gentamicin, and water deionized by using an ion exchange resin or the like. It is more effective to use deionized water in combination with mildewproofing agents or antibiotics.

It is also preferable to decrease the quantity of replenisher of the solution in the washing or stabilization tank by performing reverse osmotic film processing described in Jpn. Pat. Appln. KOKAI Publication Nos. 3-46652, 3-53246, 3-55542, 3-121448, and 3-126030. This reverse osmotic film is preferably a low-pressure reverse osmotic film.

In the processing of the present invention, it is particularly preferable to perform evaporation correction for a processing solution disclosed in JIII Journal of Technical Disclosure No. 94-4992. In particular, a method of performing correction on the basis of (equation-1) on page 2 by using the temperature and humidity information of a developing machine installation environment is preferable. Water used in evaporation correction is preferably taken from the washing replenishment tank. If this is the case, the use of deionized water as the washing replenishment water is preferable.

Processing agents described in the above-mentioned JIII Journal of Technical Disclosure, page 3, right column, line 15 to

page 4, left column, line 32 are preferably used in the present invention. As a developing machine used in the processing, a film processor described in page 3, right column, lines 22 to 28 is preferable.

Practical examples of processing agents, automatic processors, and evaporation correction methods preferably used in carrying out the present invention are described in the above-mentioned Journal of Technical Disclosure, page 5, right column, line 11 to page 7, right column, last line.

The supply form of a processing agent used in the present invention can be any of a liquid having the concentration of a solution to be used, a concentrated liquid, granules, a powder, pellets, a paste, and an emulsion. Examples of the processing agent are a liquid contained in a low-oxygen-permeability vessel disclosed in Jpn. Pat. Appln. KOKAI Publication No. 63-17453, vacuum-packed powders or granules disclosed in Jpn. Pat. Appln. KOKAI Publication Nos. 4-19655 and 4-230748, granules containing a water-soluble polymer disclosed in Jpn. Pat. Appln. KOKAI Publication No. 4-221951, pellets disclosed in Jpn. Pat. Appln. KOKAI Publication Nos. 51-61837 and 6-102628, and a paste processing agent disclosed in PCT No. 57-500485. Any of these forms can be preferably used. However, in respect of simplicity in use, the use of a liquid already prepared to have a concentration in use is preferable.

The material of vessels containing these processing agents can be any of polyethylene, polypropylene, polyvinylchloride, polyethyleneterephthalate, and nylon. These materials can be used singly or in the form of a composite material. The materials are so selected as to meet the level of a necessary oxygen permeability. Low-oxygen-permeability materials are suited to a solution such as a color developer which is readily oxidized. Practical examples are polyethyleneterephthalate and a composite material of polyethylene and nylon. The thickness of a vessel made from any of these materials is 500 to 1500  $\mu\text{m}$ . The oxygen permeability is preferably 20 ml/m<sup>2</sup>·24hrs·atm or less.

Processing solutions used for color reversal films in the present invention will be described below. The processing of color reversal films is described in detail in Known Techniques No. 6 (Apr. 1, 1991) issued by Aztec Limited Responsibility Company, page 1, line 5 to page 10, line 5, and page 15, line 8 to page 24, line 2. Any of the contents can be preferably applied.

In the processing of color reversal films, an image stabilizer is contained in a control bath or a final bath. Examples of this image stabilizer are formalin, sodium bisulfite formaldehyde, and N-methylolazoles. To preserve the work environment, the use of sodium bisulfite formaldehyde or N-methylolazoles is preferable, and N-methyloltriazole is particularly preferable among other N-methylolazoles. Also, the contents relating to the color developer, the bleaching solution, the fixer, and the washing water described in the processing of color negative films are preferably applicable to the processing of color reversal films.

Examples of color reversal film processing agents containing the above contents are an E-6 processing agent available from Eastman Kodak Co. and a CR-56 processing agent available from Fuji Photo Film Co., Ltd.

A magnetic recording layer used in the present invention will be described below.

A magnetic recording layer used in the present invention is formed by coating the surface of a support with an aqueous or organic solvent-based coating solution which is prepared by dispersing magnetic grains in a binder.

As the magnetic grains used in the present invention, it is possible to use grains of, e.g., ferromagnetic iron oxide such

as  $\gamma\text{Fe}_2\text{O}_3$ , Co-deposited  $\gamma\text{Fe}_2\text{O}_3$ , Co-deposited magnetite, Co-containing magnetite, ferromagnetic chromium dioxide, a ferromagnetic metal, a ferromagnetic alloy, Ba ferrite of a hexagonal system, Sr ferrite, Pb ferrite, and Ca ferrite. 5 Co-deposited ferromagnetic iron oxide such as Co-deposited  $\gamma\text{Fe}_2\text{O}_3$  is preferable. The grain can take the shape of any of, e.g., a needle, a rice grain, a sphere, a cube, and a plate. A specific area is preferably 20  $\text{m}^2/\text{g}$  or more, and more specifically 30  $\text{m}^2/\text{g}$  or more as  $S_{BET}$ . The saturation magnetization ( $\sigma_s$ ) of the ferromagnetic substance is preferably 10  $3.0 \times 10^4$  to  $3.0 \times 10^5$  A/m, and most preferably  $4.0 \times 10^4$  to  $2.5 \times 10^5$  A/m. A surface treatment can be performed for the ferromagnetic grains by using silica and/or alumina or an organic material. Also, the surface of the ferromagnetic grain can be treated with a silane coupling agent or a titanium coupling agent as described in Jpn. Pat. Appln. KOKAI Publication No. 6-161032. A ferromagnetic grain whose surface is coated with an inorganic or organic substance, described in Jpn. Pat. Appln. KOKAI Publication No. 4-259911 or 5-81652, also can be used.

As the binder used in the magnetic grains, it is possible to use a thermoplastic resin described in Jpn. Pat. Appln. KOKAI Publication No. 4-219569, a thermosetting resin, a radiation-curing resin, a reactive resin, an acid, an alkali or biodegradable polymer, a natural polymer (e.g., a cellulose derivative and a sugar derivative), and their mixtures.  $T_g$  of the resin is  $-40^\circ\text{C}$ . to  $300^\circ\text{C}$ ., and its weight average molecular weight is 2000 to 1,000,000. Examples are a vinyl-based copolymer, cellulose derivatives such as 15 cellulose diacetate, cellulose triacetate, celluloseacetatepropionate, celluloseacetatebutyrate, and cellulosetriacetate, an acrylic resin, and a polyvinylacetal resin. Gelatin is also preferable. Cellulosedi(tri)acetate is particularly preferable. The binder can be hardened by the 20 addition of an epoxy-, aziridine-, or isocyanate-based crosslinking agent. Examples of the isocyanate-based crosslinking agent are isocyanates such as tolylenediisocyanate, 4,4'-diphenylmethanediisocyanate, hexamethylenediisocyanate, and xylylenediisocyanate, 25 reaction products of these isocyanates and polyalcohol (e.g., a reaction product of 3 mol of tolylenediisocyanate and 1 mol of trimethylolpropane), and polyisocyanate produced by condensation of any of these isocyanates. These examples are described in Jpn. Pat. Appln. KOKAI Publication No. 35 6-59357.

As a method of dispersing the magnetic substance in the binder, as described in Jpn. Pat. Appln. KOKAI Publication No. 6-35092, the use of a kneader, a pin type mill, or an annular mill is preferable, and a combined use of these 30 apparatuses also is preferable. Dispersants described in Jpn. Pat. Appln. KOKAI Publication No. 5-88283 and other known dispersants can be used. The thickness of the magnetic recording layer is 0.1 to 10  $\mu\text{m}$ , preferably 0.2 to 5  $\mu\text{m}$ , and more preferably 0.3 to 3  $\mu\text{m}$ . The weight ratio of the 35 magnetic grains to the binder is preferably 0.5:100 to 60:100, and more preferably 1:100 to 30:100. The coating amount of the magnetic grains is 0.005 to 3  $\text{g}/\text{m}^2$ , preferably 0.01 to 2  $\text{g}/\text{m}^2$ , and more preferably 0.02 to 0.5  $\text{g}/\text{m}^2$ . The transmission yellow density of the magnetic recording layer 40 is preferably 0.01 to 0.50, more preferably 0.03 to 0.20, and most preferably 0.04 to 0.15. The magnetic recording layer used in the present invention can be formed in the whole area of, or into the shape of stripes on, the back surface of a photographic support by coating or printing. As a method 45 of coating the magnetic recording layer, it is possible to use any of an air doctor, a blade, an air knife, squeegee, impregnation, a reverse roll, a transfer roll, gravure, kiss,

cast, spray, dip, a bar, and extrusion. A coating solution described in Jpn. Pat. Appln. KOKAI Publication No. 5-341436 is preferable.

The magnetic recording layer can be given a lubricating property improving function, a curling adjusting function, an antistatic function, an adhesion preventing function, and a head polishing function. Alternatively, another functional layer can be formed and these functions can be given to that layer. A polishing agent in which at least one type of grains are aspherical inorganic grains having a Mohs hardness of 5 or more is preferable. The composition of the aspherical inorganic grain is preferably an oxide such as aluminum oxide, chromium oxide, silicon dioxide, titanium dioxide, and silicon carbide, a carbide such as silicon carbide and titanium carbide, or a fine powder of diamond. The surfaces of the grains constituting these polishing agents can be treated with a silane coupling agent or a titanium coupling agent. These grains can be added to the magnetic recording layer or overcoated (as, e.g., a protective layer or a lubricant layer) on the magnetic recording layer. The binder used together with the grains can be any of those described above and is preferably the same binder as in the magnetic recording layer. Light-sensitive materials having the magnetic recording layer are described in U.S. Pat. Nos. 5,336,589, 5,250,404, 5,229,259, and 5,215,874, and European Patent No. 466,130.

A polyester support used in the present invention will be described below. Details of the polyester support and light-sensitive materials, processing, cartridges, and examples (to be described later) are described in Journal of Technical Disclosure No. 94-6023 (JIII; Mar. 15, 1994). Polyester used in the present invention is formed by using diol and aromatic dicarboxylic acid as essential components. Examples of the aromatic dicarboxylic acid are 2,6-, 1,5-, 1,4-, and 2,7-naphthalenedicarboxylic acids, terephthalic acid, isophthalic acid, and phthalic acid. Examples of the diol are diethylene glycol, triethylene glycol, cyclohexanedimethanol, bisphenol A, and bisphenol. Examples of the polymer are homopolymers such as polyethyleneterephthalate, polyethylenenaphthalate, and polycyclohexanedimethanolterephthalate. Polyester containing 50 to 100 mol % of 2,6-naphthalenedicarboxylic acid is particularly preferable. Polyethylene-2,6-naphthalate is most preferable among other polymers. The average molecular weight ranges between about 5,000 and 200,000. Tg of the polyester of the present invention is 50° C. or higher, preferably 90° C. or higher.

To give the polyester support a resistance to curling, the polyester support is heat-treated at a temperature of 40° C. to less than Tg, more preferably Tg—20° C. to less than Tg. The heat treatment can be performed at a fixed temperature within this range or can be performed together with cooling. The heat treatment time is 0.1 to 1500 hr, more preferably 0.5 to 200 hr. The heat treatment can be performed for a roll-like support or while a support is conveyed in the form of a web. The surface shape also can be improved by forming undulations (e.g., coating conductive inorganic fine grains such as SnO<sub>2</sub> or Sb<sub>2</sub>O<sub>5</sub> grains) on the surface. It is desirable to knurl and slightly raise the end portion, thereby preventing the cut edge of the core portion from being photographed. These heat treatments can be performed in any stage after support film formation, after surface treatment, after back layer coating (e.g., an antistatic agent or a lubricating agent), and after undercoating. A preferable timing is after the antistatic agent is coated.

An ultraviolet absorbent can be incorporated into this polyester. Also, light piping can be prevented by incorpo-

rating dyes or pigments such as Diaresin manufactured by Mitsubishi Kasei Corp. or Kayaset manufactured by NIPPON KAYAKU CO. LTD. commercially available for polyester.

In the present invention, it is preferable to perform a surface treatment in order to adhere the support and the light-sensitive material constituting layers. Examples of the surface treatment are surface activation treatments such as a chemical treatment, a mechanical treatment, a corona discharge treatment, a flame treatment, an ultraviolet treatment, a high-frequency treatment, a glow discharge treatment, an active plasma treatment, a laser treatment, a mixed acid treatment, and an ozone oxidation treatment. Among other surface treatments, the ultraviolet irradiation treatment, the flame treatment, the corona treatment, and the glow treatment are preferable.

The undercoating layer can consist of a single layer or two or more layers. Examples of the undercoating layer binder are copolymers formed by using, as the starting material, a monomer selected from vinylchloride, vinylidenechloride, butadiene, methacrylic acid, acrylic acid, itaconic acid, and maleic anhydride. Other examples are polyethyleneimine, an epoxy resin, grafted gelatin, nitrocellulose, and gelatin. Resorcin and p-chlorophenol are examples of a compound which swells the support. Examples of a gelatin hardener added to the undercoating layer are chromium salt (e.g., chromium alum), aldehydes (e.g., formaldehyde and glutaraldehyde), isocyanates, an active halogen compound (e.g., 2,4-dichloro-6-hydroxys-triazine), an epichlorohydrin resin, and an active vinylsulfone compound. SiO<sub>2</sub>, TiO<sub>2</sub>, inorganic fine grains, or polymethylmethacrylate copolymer fine grains (0.01 to 10  $\mu$ m) can also be contained as a matting agent.

In the present invention, antistatic agents are preferably used. Examples of these antistatic agents are carboxylic acid and carboxylate, a macromolecule containing sulfonate, a cationic macromolecule, and an ionic surfactant compound.

As the antistatic agent, it is most preferable to use fine grains of at least one crystalline metal oxide selected from ZnO, TiO<sub>2</sub>, SnO<sub>2</sub>, Al<sub>2</sub>O<sub>3</sub>, In<sub>2</sub>O<sub>3</sub>, SiO<sub>2</sub>, MgO, BaO, MoO<sub>3</sub>, and V<sub>2</sub>O<sub>5</sub> and having a volume resistivity of 10<sup>7</sup>  $\Omega$ ·cm or less, more preferably 10<sup>5</sup>  $\Omega$ ·cm or less and a grain size of 0.001 to 1.0  $\mu$ m, fine grains of composite oxides (e.g., Sb, P, B, In, S, Si, and C) of these metal oxides, fine grains of sol metal oxides, or fine grains of composite oxides of these sol metal oxides. The content in the light-sensitive material is preferably 5 to 500 mg/m<sup>2</sup>, and most preferably 10 to 350 mg/m<sup>2</sup>. The ratio of a conductive crystalline oxide or its composite oxide to the binder is preferably 1/300 to 100/1, and more preferably 1/100 to 100/5.

The light-sensitive material of the present invention preferably has a slip property. Slip agent-containing layers are preferably formed on the surfaces of both a light-sensitive layer and a back layer. A preferable slip property is 0.01 to 0.25 as a coefficient of kinetic friction. This represents a value obtained when a stainless steel sphere 5 mm in diameter is conveyed at a speed of 60 cm/min (25° C., 60%RH). In this evaluation, a value of nearly the same level is obtained even when the surface of a light-sensitive layer is used as the sample to be measured.

Examples of the slip agent usable in the present invention are polyorganocyloxane, higher fatty acid amide, higher fatty acid metal salt, and esters of higher fatty acid and higher alcohol. As the polyorganocyloxane, it is possible to use polydimethylcyloxane, polydiethylcyloxane, polystyrylmethylcyloxane, and polymethylphenylcyloxane. A layer to which the slip agent is added is preferably the

outermost emulsion layer or the back layer. Polydimethylcylohexane or ester having a long-chain alkyl group is particularly preferable.

The light-sensitive material of the present invention preferably contains a matting agent. The matting agent can be added to either the emulsion surface or the back surface and is most preferably added to the outermost emulsion layer. The matting agent can be either soluble or insoluble in processing solutions, and the use of both types of matting agents is preferable. Preferable examples are polymethylmethacrylate grains, poly(methylmethacrylate/methacrylic acid=9/1 or 5/5 (molar ratio)) grains, and polystyrene grains. The grain size is preferably 0.8 to 10  $\mu\text{m}$ , and a narrow grain size distribution is preferable. It is preferable that 90% or more of all grains have grain sizes 0.9 to 1.1 times the average grain size. To increase the matting property, it is preferable to simultaneously add fine grains with a grain size of 0.8  $\mu\text{m}$  or smaller. Examples are polymethylmethacrylate grains (0.2  $\mu\text{m}$ ), poly(methylmethacrylate/methacrylic acid=9/1 (molar ratio, 0.3  $\mu\text{m}$ )) grains, polystyrene grains (0.25  $\mu\text{m}$ ), and colloidal silica grains (0.03  $\mu\text{m}$ ).

A film magazine used in the present invention will be described below. The principal material of the cartridge used in the present invention can be a metal or synthetic plastic.

Preferable plastic materials are polystyrene, polyethylene, polypropylene, and polyphenylether. The cartridge of the present invention can also contain various antistatic agents. For this purpose, carbon black, metal oxide grains, nonion-, anion-, cation-, and betaine-based surfactants, or a polymer can be preferably used. These antistatic cartridges are described in Jpn. Pat. Appln. KOKAI Publication Nos. 1-312537 and 1-312538. It is particularly preferable that a resistance at 25° C. and 25%RH be  $10^{12} \Omega$  or less. Commonly, plastic cartridges are manufactured by using plastic into which carbon black or pigments are incorporated in order to give a light-shielding property. The cartridge size can be a presently available 135 size. To miniaturize cameras, it is effective to decrease the diameter of a 25-mm cartridge of 135 size to 22 mm or less. The volume of a cartridge case is 30  $\text{cm}^3$  or less, preferably 25  $\text{cm}^3$  or less. The weight of plastic used in the cartridge and the cartridge case is preferably 5 to 15 g.

Furthermore, a cartridge which feeds a film by rotating a spool can be used in the present invention. It is also possible to use a structure in which a film leader is housed in a cartridge main body and fed through a port of the cartridge to the outside by rotating a spool shaft in the film feed direction. These structures are disclosed in U.S. Pat. Nos. 4,834,306 and 5,226,613. Photographic films used in the present invention can be so-called raw films before being developed or developed photographic films. Also, raw and developed photographic films can be accommodated in the same new cartridge or in different cartridges.

## EXAMPLES

The present invention will be described in more detail below by way of its examples. However, the present invention is not limited to these examples.

### Example 1

#### 1) Support

A support used in this example was formed as follows. 100 parts by weight of a commercially available polyethylene-2,6-naphthalate polymer and 2 parts by weight of Tinuvin P.326 (manufactured by Ciba-Geigy Co.) as an ultraviolet absorbent were dried by a conventional method, melted at 300° C., and extruded from a T-die. The resultant

material was longitudinally oriented by 3.0 times at 140° C., laterally oriented by 3.0 times at 130° C., and thermally fixed at 250° C. for 6 sec. The result was a 90- $\mu\text{m}$  thick PEN film.

5 A portion of the PEN film was wound around a stainless steel core 20 cm in diameter and given a thermal history of 110° C. and 48 hr.

#### 2) Coating of undercoat layer

The two surfaces of the support were subjected to corona discharge, UV discharge, glow discharge, and a flame treatment, and coated with an undercoat solution having the composition described below, thereby forming undercoat layers on sides at a high temperature upon orientation. The corona discharge processing was performed for a 30-cm wide support at 20 m/min by using a solid state color processor 6KVA manufactured by Pillar Co. It was found from the readings of the current and voltage that processing of 0.375 KV·A·min/m<sup>2</sup> was performed for the object to be processed. During the processing, the discharge frequency was 9.6 KHz, and the gap clearance between the electrode and the dielectric roll was 1.6 mm. The UV discharge processing was done by heating the support at 75° C. The glow discharge processing was done by irradiating the support at 3000 W for 30 sec by using a columnar electrode.

|                                                                             |        |
|-----------------------------------------------------------------------------|--------|
| Gelatin                                                                     | 3 g    |
| Distilled water                                                             | 25 ml  |
| Sodium $\alpha$ -sulfo-di-2-ethylhexylsuccinate                             | 0.05 g |
| Formaldehyde                                                                | 0.02 g |
| Salicylic acid                                                              | 0.1 g  |
| Diacetylcellulose                                                           | 0.5 g  |
| p-chlorophenol                                                              | 0.5 g  |
| Resorcin                                                                    | 0.5 g  |
| Cresol                                                                      | 0.5 g  |
| $(\text{CH}_2=\text{CHSO}_2\text{CH}_2\text{CH}_2\text{NHCO})_3\text{CH}_2$ | 0.2 g  |
| Aziridine three-time molar adduct of trimethylolpropane                     | 0.2 g  |
| Three-time molar adduct of trimethylolpropane-toluenediisocyanate           | 0.2 g  |
| Methanol                                                                    | 15 ml  |
| Acetone                                                                     | 85 ml  |
| Formaldehyde                                                                | 0.01 g |
| Acetic acid                                                                 | 0.01 g |
| Concentrated hydrochloric acid                                              | 0.01 g |

#### 3) Coating of back layers

On one surface of the undercoated support, an antistatic layer, a magnetic recording layer, and a slip layer having the following compositions were coated as back layers.

##### 3-1) Coating of antistatic layer

###### 3-1-1) Preparation of conductive fine grain dispersion (dispersion of tin oxide-antimony oxide composite material)

50 230 parts by weight of stannic chloride hydrate and 23 parts by weight of antimony trichloride were dissolved in 3000 parts by weight of ethanol to prepare a uniform solution. An aqueous 1 N sodium hydroxide solution was dropped into the resultant solution until the pH of the solution became 3, thereby obtaining a co-precipitate of colloidal stannic oxide and antimony oxide. The resultant co-precipitate was left to stand at 50° C. for 24 hr to obtain a reddish brown colloidal precipitate.

55 The reddish brown colloidal precipitate was separated by centrifugal separation. To remove excess ion, water is added to the precipitate and the precipitate was washed with the water by centrifugal separation. This operation was repeated three times to remove excess ion.

60 65 200 parts by weight of the colloidal precipitate from which excess ion was removed were again dispersed in 1500 parts by weight of water, and the dispersion was sprayed into a sintering furnace heated to 650° C. The result was a bluish

fine grain powder with an average grain size of  $0.005\text{ }\mu\text{m}$  of a tin oxide-oxide antimony composite material. The specific resistance of this fine grain powder was  $5\text{ }\Omega\text{-cm}$ .

The pH of a solution mixture of 40 parts by weight of the fine grain powder and 60 parts by weight of water was adjusted to 7.0, and the mixture was coarsely dispersed by using a stirrer. Thereafter, the coarse dispersion was dispersed by a horizontal sand mill (Dynomill (tradename); manufactured by WILLYA. BACHOFENAG) until the retention time was 30 min. The average grain size of the secondary aggregate was about  $0.04\text{ }\mu\text{m}$ .

### 3-1-2) Coating of conductive layer

A conductive layer having the following composition was coated such that the dry film thickness was  $0.2\text{ }\mu\text{m}$ , and dried at  $115^\circ\text{ C}$ . for 60 sec.

|                                                     |                     |
|-----------------------------------------------------|---------------------|
| Conductive fine grain dispersion prepared in 3-1-1) | 20 parts by weight  |
| Gelatin                                             | 2 parts by weight   |
| Water                                               | 27 parts by weight  |
| Methanol                                            | 60 parts by weight  |
| p-chlorophenol                                      | 0.5 part by weight  |
| Resorcin                                            | 2 parts by weight   |
| Polyoxyethylenenonylphenylether                     | 0.01 part by weight |

The resistance of the resultant conductive film was  $10^{8.0}$  (100 v), i.e., the conductive film had excellent antistatic properties.

### 3-2) Coating of magnetic recording layer

1100 g of magnetic substance Co-deposited  $\gamma\text{-Fe}_2\text{O}_3$  (needles having a major axis of  $0.14\text{ }\mu\text{m}$  and a minor axis of  $0.03\text{ }\mu\text{m}$ , specific area  $41\text{ m}^2/\text{g}$ , saturation magnetization 89 emu/g, the surface was treated with 2 wt % of  $\text{Fe}_2\text{O}_3$  by using aluminum oxide and silicon oxide, coercive force 930 Oe,  $\text{Fe}^{+2}/\text{Fe}^{+3}=6/94$ ), 220 g of water, and 150 g of a silane coupling agent made from polyoxyethylenenopropyltrimethoxysilane (polymerization degree 16), and the mixture was well kneaded in an open kneader for 3 hr. The resultant coarsely dispersed viscous solution was dried at  $70^\circ\text{ C}$ . for 24 hr to remove water. Thereafter, the resultant material was heated at  $110^\circ\text{ C}$ . for a whole day and night to form surface-treated magnetic grains.

The following composition was again kneaded by the open kneader.

|                                                 |        |
|-------------------------------------------------|--------|
| Above-mentioned surface-treated magnetic grains | 1000 g |
| Diacetylcellulose                               | 17 g   |
| Methylethylketone                               | 100 g  |
| Cyclohexanone                                   | 100 g  |

Furthermore, the following composition was finely dispersed at 200 rpm for 4 hr by a sand mill ( $\frac{1}{4}$  G).

|                                 |       |
|---------------------------------|-------|
| Above-mentioned kneaded product | 100 g |
| Diacetylcellulose               | 60 g  |
| Methylethylketone               | 300 g |
| Cyclohexanone                   | 300 g |

Additionally, 20 wt % of diacetylcellulose and a three-time molar adduct of trimethylolpropane-toluenediisocyanate as a hardener were added to the binder. The resultant solution was diluted by equal quantities of methylethylketone and cyclohexanone so that the viscosity of the solution was about 80 cp. Coating was done on the conductive layer by using a bar coater so that the film thickness was  $1.2\text{ }\mu\text{m}$  and the amount of the magnetic

substance was  $0.6\text{ g/m}^2$ .  $10\text{ mg/m}^2$  of silica grains ( $0.3\text{ }\mu\text{m}$ ) were added as a matting agent, and  $10\text{ mg/m}^2$  of aluminum oxide ( $0.5\text{ }\mu\text{m}$ ) were added as a polishing agent. Drying was performed at  $115^\circ\text{ C}$ . for 6 min (all rollers and conveyors in the drying zone were at  $115^\circ\text{ C}$ .).

An increase in the color density of  $D^8$  of the magnetic recording layer measured by using a blue filter in status M of X-light was about 0.1. The saturation magnetization moment, coercive force, and squareness ratio of the magnetic recording layer were  $4.2\text{ emu/m}^2$ , 923 Oe, and 65%, respectively.

### 3-3) Preparation of slip layer

A solution having the following composition was coated such that the solid coating amounts of the compounds were as follows, and dried at  $110^\circ\text{ C}$ . for 5 min to obtain a slip layer.

|    |                                                                                                                                                                                                                                           |                                                                    |
|----|-------------------------------------------------------------------------------------------------------------------------------------------------------------------------------------------------------------------------------------------|--------------------------------------------------------------------|
| 20 | Diacetylcellulose<br>$\text{C}_6\text{H}_{13}\text{CH}(\text{OH})\text{C}_{10}\text{H}_{20}\text{COOC}_{40}\text{H}_{81}$ (compound a)<br>$\text{C}_{50}\text{H}_{101}\text{O}(\text{CH}_2\text{CH}_2\text{O})_{16}\text{H}$ (compound b) | 25 mg/m <sup>2</sup><br>6 mg/m <sup>2</sup><br>9 mg/m <sup>2</sup> |
|----|-------------------------------------------------------------------------------------------------------------------------------------------------------------------------------------------------------------------------------------------|--------------------------------------------------------------------|

Note that the compound a/compound b (6:9) mixture was dissolved in an xylene-propyleneglycolmonomethylether (volume ratio 1:1) solvent by heating to  $105^\circ\text{ C}$ . The resultant solution was injected into a tenfold amount of propyleneglycolmonomethylether ( $25^\circ\text{ C}$ .) to prepare a fine dispersion. The dispersion was diluted in a fivefold amount of acetone, and the diluted solution was redispersed by a high-pressure homogenizer (200 atm) and formed into a dispersion (average grain size  $0.01\text{ }\mu\text{m}$ ) before being added.

The resultant slip layer was found to have excellent characteristics; that is, the coefficient of kinetic friction was 0.06 (5 mmø stainless steel hard sphere, load 100 g, speed 6 cm/min), and the coefficient of static friction was 0.07 (clip method). Also, the coefficient of kinetic friction between an emulsion surface (to be described later) and the slip layer was 0.12.

### 4) Coating of sensitive layers

On the side away from the back layers formed as above, a plurality of layers having the following compositions were coated to manufacture a color negative film. The film is called a sample 101.

#### (Compositions of light-sensitive layers)

The main materials used in the individual layers are classified as follows.

|                      |                                   |
|----------------------|-----------------------------------|
| ExC: Cyan coupler    | UV : Ultraviolet absorbent        |
| ExM: Magenta coupler | HBS: High-boiling organic solvent |
| ExY: Yellow coupler  | H : Gelatin hardener              |
| ExS: Sensitizing dye |                                   |

The number corresponding to each component indicates the coating amount in units of  $\text{g/m}^2$ . The coating amount of a silver halide is represented by the amount of silver. The coating amount of each sensitizing dye is represented in units of mols per mol of a silver halide in the same layer. (Sample 101)

1st layer (1st antihalation layer)

|                        |             |
|------------------------|-------------|
| Black colloidal silver | silver 0.08 |
| Gelatin                | 58          |

## 2nd layer (2nd antihalation layer)

|                            |        |                      |
|----------------------------|--------|----------------------|
| Black colloidal silver     | silver | 0.09                 |
| Gelatin                    |        | 0.64                 |
| ExM-1                      |        | 0.12                 |
| ExF-1                      |        | $2.0 \times 10^{-3}$ |
| Solid dispersion dye ExF-2 |        | 0.030                |
| Solid dispersion dye ExF-3 |        | 0.040                |
| HBS-1                      |        | 0.15                 |
| HBS-2                      |        | 0.02                 |

## 7th layer (Interlayer)

|                            |  |       |
|----------------------------|--|-------|
| Cpd-1                      |  | 0.060 |
| Solid dispersion dye ExF-4 |  | 0.030 |
| HBS-1                      |  | 0.040 |
| Polyethylacrylate latex    |  | 0.15  |
| Gelatin                    |  | 1.10  |

## 3rd layer (Interlayer)

|                         |  |      |
|-------------------------|--|------|
| ExC-2                   |  | 0.05 |
| Polyethylacrylate latex |  | 0.20 |
| Gelatin                 |  | 0.47 |

## 4th layer (Low-speed red-sensitive emulsion layer)

|                               |        |                      |
|-------------------------------|--------|----------------------|
| Silver iodobromide emulsion A | silver | 0.23                 |
| Silver iodobromide emulsion B | silver | 0.26                 |
| silver iodobromide emulsion C | silver | 0.10                 |
| ExS-1                         |        | $4.3 \times 10^{-4}$ |
| ExS-2                         |        | $1.8 \times 10^{-5}$ |
| ExS-3                         |        | $5.9 \times 10^{-4}$ |
| ExC-1                         |        | 0.33                 |
| ExC-2                         |        | 0.02                 |
| ExC-3                         |        | 0.06                 |
| ExC-4                         |        | 0.014                |
| ExC-5                         |        | 0.021                |
| ExC-6                         |        | 0.002                |
| Cpd-2                         |        | 0.033                |
| HBS-1                         |        | 0.13                 |
| Gelatin                       |        | 1.37                 |

## 5th layer (Medium-speed red-sensitive emulsion layer)

|            |        |                      |
|------------|--------|----------------------|
| Emulsion C | silver | 0.15                 |
| Emulsion D | silver | 0.46                 |
| ExS-1      |        | $4.0 \times 10^{-4}$ |
| ExS-2      |        | $2.1 \times 10^{-5}$ |
| ExS-3      |        | $5.7 \times 10^{-4}$ |
| ExC-1      |        | 0.23                 |
| ExC-2      |        | 0.02                 |
| ExC-3      |        | 0.03                 |
| ExC-4      |        | 0.017                |
| ExC-5      |        | 0.02                 |
| ExC-6      |        | 0.001                |
| Cpd-4      |        | 0.030                |
| Cpd-2      |        | 0.05                 |
| HBS-1      |        | 0.10                 |
| Gelatin    |        | 0.93                 |

## 6th layer (High-speed red-sensitive emulsion layer)

|                               |        |                      |
|-------------------------------|--------|----------------------|
| Silver iodobromide emulsion E | silver | 1.47                 |
| ExS-1                         |        | $2.8 \times 10^{-4}$ |
| ExS-2                         |        | $1.2 \times 10^{-5}$ |
| ExS-3                         |        | $4.1 \times 10^{-4}$ |
| ExC-1                         |        | 0.12                 |
| ExC-3                         |        | 0.10                 |
| ExC-4                         |        | 0.037                |
| ExC-6                         |        | 0.003                |
| ExC-7                         |        | 0.010                |
| Cpd-2                         |        | 0.059                |
| Cpd-4                         |        | 0.020                |
| HBS-1                         |        | 0.22                 |
| HBS-2                         |        | 0.050                |
| Gelatin                       |        | 1.40                 |

## 5,985,531

## 10 8th layer (Low-speed green-sensitive emulsion layer)

|                               |        |                      |
|-------------------------------|--------|----------------------|
| Silver iodobromide emulsion F | silver | 0.22                 |
| Silver iodobromide emulsion G | silver | 0.35                 |
| ExS-7                         |        | $6.2 \times 10^{-4}$ |
| ExS-8                         |        | $1.4 \times 10^{-4}$ |
| ExS-4                         |        | $2.7 \times 10^{-5}$ |
| ExS-5                         |        | $7.0 \times 10^{-5}$ |
| ExS-6                         |        | $2.7 \times 10^{-4}$ |
| ExM-3                         |        | 0.38                 |
| ExM-4                         |        | 0.084                |
| ExC-4                         |        | 0.002                |
| ExY-1                         |        | 0.040                |
| ExY-5                         |        | 0.003                |
| HBS-1                         |        | 0.30                 |
| HBS-3                         |        | 0.015                |
| Cpd-4                         |        | 0.010                |
| Gelatin                       |        | 1.07                 |

## 9th layer (Medium-speed green-sensitive emulsion layer)

|                               |        |                       |
|-------------------------------|--------|-----------------------|
| Silver iodobromide emulsion G | silver | 0.56                  |
| Silver iodobromide emulsion H | silver | 0.56                  |
| ExS-4                         |        | $5.6 \times 10^{-5}$  |
| ExS-7                         |        | $1.09 \times 10^{-3}$ |
| ExS-8                         |        | $2.5 \times 10^{-4}$  |
| ExC-4                         |        | 0.004                 |
| ExC-8                         |        | 0.002                 |
| ExM-3                         |        | 0.126                 |
| ExM-4                         |        | 0.035                 |
| ExY-1                         |        | 0.008                 |
| ExY-4                         |        | 0.010                 |
| ExY-5                         |        | 0.0050                |
| Cpd-4                         |        | 0.011                 |
| HBS-1                         |        | 0.13                  |
| HBS-3                         |        | $4.4 \times 10^{-3}$  |
| Gelatin                       |        | 1.02                  |

## 45 10th layer (High-speed green-sensitive emulsion layer)

|                               |        |                      |
|-------------------------------|--------|----------------------|
| Silver iodobromide emulsion I | silver | 1.34                 |
| ExS-4                         |        | $4.6 \times 10^{-5}$ |
| ExS-7                         |        | $5.5 \times 10^{-4}$ |
| ExS-8                         |        | $1.2 \times 10^{-4}$ |
| ExC-9                         |        | 0.019                |
| ExM-1                         |        | 0.010                |
| ExM-2                         |        | 0.030                |
| ExM-5                         |        | 0.0070               |
| ExM-6                         |        | 0.0050               |
| Cpd-3                         |        | 0.015                |
| Cpd-4                         |        | 0.031                |
| HBS-1                         |        | 0.25                 |
| Polyethylacrylate latex       |        | 0.15                 |
| Gelatin                       |        | 1.29                 |

## 60 11th layer (Yellow filter layer)

|                            |        |       |
|----------------------------|--------|-------|
| Yellow colloidal silver    | silver | 0.030 |
| Cpd-1                      |        | 0.10  |
| Solid dispersion dye ExF-5 |        | 0.060 |
| Solid dispersion dye ExF-6 |        | 0.060 |

-continued

|                       |       |
|-----------------------|-------|
| Oil-soluble dye ExF-7 | 0.010 |
| HBS-1                 | 0.60  |
| Gelatin               | 0.69  |

12th layer (Low-speed blue-sensitive emulsion layer)

|                               |                      |
|-------------------------------|----------------------|
| Silver iodobromide emulsion J | silver 0.09          |
| Silver iodobromide emulsion K | silver 0.10          |
| Silver iodobromide emulsion L | silver 0.25          |
| ExS-9                         | $8.4 \times 10^{-4}$ |
| ExC-9                         | 0.01                 |
| ExC-8                         | $7.0 \times 10^{-3}$ |
| ExC-6                         | 0.024                |
| ExY-1                         | 0.050                |
| ExY-2                         | 0.75                 |
| ExY-3                         | 0.40                 |
| ExY-4                         | 0.040                |
| Cpd-2                         | 0.10                 |
| Cpd-4                         | 0.01                 |
| Cpd-3                         | $4.0 \times 10^{-3}$ |
| HBS-1                         | 0.28                 |
| Gelatin                       | 2.45                 |

5

-continued

|         |                      |
|---------|----------------------|
| HBS-4   | $5.0 \times 10^{-2}$ |
| Gelatin | 1.99                 |

15th layer (2nd protective layer)

|                                   |      |
|-----------------------------------|------|
| H-1                               | 0.40 |
| B-1 (diameter 1.7 $\mu\text{m}$ ) | 0.06 |
| B-2 (diameter 1.7 $\mu\text{m}$ ) | 0.09 |
| B-3                               | 0.13 |
| ES-1                              | 0.20 |
| Gelatin                           | 0.74 |

15 In addition to the above components, to improve the storage stability, processability, resistance to pressure, anti-septic and mildewproofing properties, antistatic properties, and coating properties, the individual layers contained W-1 to W-3, B-4 to B-6, F-1 to F-18, iron salt, lead salt, gold salt, platinum salt, palladium salt, iridium salt, and rhodium salt.

20 TABLE 1 below shows the average AgI contents and the grain sizes of the emulsions A to M used in the manufacture of the sample 101.

TABLE 1

| Emulsion | Average AgI content (%) | Equivalent sphere diameter of average grain size ( $\mu\text{m}$ ) | Variation coefficient according to grain size (%) | Equivalent circle diameter of projected area ( $\mu\text{m}$ ) | Diameter/thickness ratio | Flatness |
|----------|-------------------------|--------------------------------------------------------------------|---------------------------------------------------|----------------------------------------------------------------|--------------------------|----------|
| A        | 2.5                     | 0.37                                                               | 10                                                | 0.40                                                           | 2.4                      | 14       |
| B        | 3.1                     | 0.40                                                               | 18                                                | 0.51                                                           | 3.2                      | 20       |
| C        | 5.0                     | 0.55                                                               | 20                                                | 0.86                                                           | 6.2                      | 45       |
| D        | 5.4                     | 0.66                                                               | 23                                                | 1.10                                                           | 7.0                      | 45       |
| E        | 4.2                     | 0.81                                                               | 19                                                | 1.20                                                           | 6.9                      | 40       |
| F        | 2.7                     | 0.37                                                               | 19                                                | 0.58                                                           | 3.2                      | 18       |
| G        | 3.3                     | 0.42                                                               | 18                                                | 0.80                                                           | 5.9                      | 44       |
| H        | 4.0                     | 0.61                                                               | 20                                                | 1.10                                                           | 6.5                      | 38       |
| I        | 4.2                     | 0.80                                                               | 20                                                | 1.09                                                           | 7.1                      | 46       |
| J        | 3.2                     | 0.35                                                               | 19                                                | 0.56                                                           | 6.9                      | 85       |
| K        | 3.3                     | 0.34                                                               | 21                                                | 0.56                                                           | 7.1                      | 90       |
| L        | 6.0                     | 0.62                                                               | 20                                                | 0.83                                                           | 8.9                      | 95       |
| M        | 6.3                     | 1.00                                                               | 19                                                | 1.30                                                           | 6.0                      | 28       |
| N        | 1.0                     | 0.07                                                               | 15                                                | —                                                              | 1.0                      | —        |

13th layer (High-speed blue-sensitive emulsion layer)

|                               |                      |
|-------------------------------|----------------------|
| Silver iodobromide emulsion M | silver 0.51          |
| ExS-9                         | $3.1 \times 10^{-4}$ |
| ExY-2                         | 0.070                |
| ExY-3                         | 0.070                |
| ExY-4                         | 0.0050               |
| Cpd-2                         | 0.019                |
| Cpd-3                         | $1.0 \times 10^{-3}$ |
| Cpd-4                         | 0.02                 |
| HBS-1                         | 0.070                |
| Gelatin                       | 0.50                 |

14th layer (1st protective layer)

|                               |                      |
|-------------------------------|----------------------|
| Silver iodobromide emulsion N | silver 0.10          |
| UV-1                          | 0.13                 |
| UV-2                          | 0.10                 |
| UV-3                          | 0.16                 |
| UV-4                          | 0.025                |
| ExF-8                         | 0.001                |
| ExF-9                         | 0.002                |
| HBS-1                         | $5.0 \times 10^{-2}$ |

45 In TABLE 1,

(1) The emulsions J to L were subjected to reduction sensitization during grain preparation by using thiourea dioxide and thiosulfonic acid in accordance with the examples in Jpn. Pat. Appln. KOKAI Publication No. 2-191938.

50 (2) The emulsions C to E, G to I, and M were subjected to gold sensitization, sulfur sensitization, and selenium sensitization in the presence of the spectral sensitizing dyes described in the individual light-sensitive layers and sodium thiocyanate in accordance with the examples in Jpn. Pat. Appln. KOKAI Publication No. 3-237450.

55 (3) The tabular grains were prepared by using low-molecular weight gelatin in accordance with the examples in Jpn. Pat. Appln. KOKAI Publication No. 1-158426.

(4) Dislocation lines as described in Jpn. Pat. Appln. 60 KOKAI Publication No. 3-237450 were observed in tabular grains when a high-voltage electron microscope was used.

(5) The emulsions A to E, G, H, and J to L contained optimum amounts of Rh, Ir, and Fe.

Also, assuming that the average equivalent circle diameter of the projected areas of tabular grains is  $D_c$  and the average thickness of the tabular grains is  $t$ , the flatness is represented by flatness =  $D_c/t^2$ .

75

## Preparation of dispersions of organic solid dispersion dyes

The dye ExF-2 described below was dispersed by the following method. That is, 21.7 ml of water, 3 ml of a 5% aqueous solution of p-octylphenoxyethoxyethoxyethanesulfonic acid soda, and 0.5 g of a 5% aqueous solution of p-octylphenoxypropoxyethoxyethyleneether (polymerization degree 10) were placed in a 700-ml pot mill, and 5.0 g of the dye ExF-2 and 500 ml of zirconium oxide beads (diameter 1 mm) were added to the mill. The contents were dispersed for 2 hr. This dispersion was done by using a BO type oscillating ball mill manufactured by Chuo Koki K.K. The dispersion was removed from the mill and added to 8 g of

76

a 12.5% aqueous solution of gelatin. The beads were removed from the resultant material by filtration, obtaining a gelatin dispersion of the dye. The average grain size of the fine dye grains was  $0.44 \mu\text{m}$ .

Following the same procedure as above, solid dispersions of the dyes ExF-3, ExF-4, and ExF-6 described below were obtained. The average grain sizes of these fine dye grains were 0.24, 0.45, and 0.52  $\mu\text{m}$ , respectively. ExF-5 was dispersed by a micro-precipitation dispersion method described in Example 1 of EP 549,489A. The average grain size was found to be 0.06  $\mu\text{m}$ .

The compounds used in the formation of the above layers are presented below.

### ExC-1



ExC-2



### ExC-3



### ExC-4



-continued



ExC-5



ExC-6



ExC-8



-continued

ExC-9



ExM-2



ExM-3



### ExM=4



ExM-5



ExM-6



ExY-1



-continued



ExY-2



ExY-3



ExY-4



ExY-5



ExF-1

-continued



ExF-2



ExF-3



ExF-4



ExF-5



ExF-6



ExF-7



-continued

ExF-8



ExF-9



Cpd-1



Cpd-2



Cpd-3



Cpd-4



UV-1





Tricresylphosphate

Di-n-butylphthalate



Tri(2-ethylhexyl)phosphate



-continued



ExS-4



ExS-5



ExS-6



ExS-7



ExS-8



ExS-9

S-1



H-1



B-1



x/y = 10/90

-continued



$$x/y = 40/60$$

94

B-3



B-3



B 4



x/v = 70/30

B 5



(mol. wt. about 10,000)

B-6



W-1



$$n = 2-4$$

W-2



W-3



F-1



F-3



E-4



E-5



F-6



F-7



E-8



F-9



E-10



-continued



98

E-11



F-12



F-13



E 14



E 15



E-16



E-18

Samples 102 to 112 (see TABLE 2 below) were formed by replacing the coupler ExC-4 used in the fourth, fifth, and sixth layers of the sample 101 with comparative compounds (1) to (3) presented below and the compounds of the present invention. 50

Note that the addition amounts of the couplers used were so adjusted that the cyan image gradation of each sample was equal to that of the sample 101. 55

Comparative compound (1): Compound (4) disclosed in <sup>60</sup> JP-A-5-313322



99

Comparative compound (2): Compound (1) disclosed in JP-A-5-313322



Comparative compound (3): Compound (2) disclosed in JP-A-5-313322



Subsequently, each sample was cut into 24 mm wide and 160 cm long, and two square perforations of 2 mm side were formed at an interval of 5.8 mm in a position 0.7 mm away from one side in the longitudinal direction of the sample. These pairs of perforations were formed at intervals of 32 mm, and the film was accommodated in a plastic film cartridge explained in FIGS. 1 to 7 of U.S. Pat. No. 5,296,887.

An FM signal was recorded between the perforations at a feed speed of 100 mm/s from the magnetic recording layer coated side of these samples by using a head having a head gap of 5  $\mu\text{m}$  and the number of turns of 2000 and capable of input and output. After the FM signal was recorded, exposure corresponding to the property evaluations described below was given from the light-sensitive layer side, and the following development was performed to evaluate the individual properties. In each development processing, running processing was performed (until the accumulated replenisher volume of the color developer was three times the tank volume) by using a processing machine for motion picture film.

100

The processing steps and the compositions of the processing solutions were as follows.

|        |                   | (Processing steps) |              |       |      |
|--------|-------------------|--------------------|--------------|-------|------|
| Step   | Time              | Tempera-           | Quantity of  |       |      |
| volume |                   | ture               | replenisher* | Tank  |      |
| 10     | Color development | 3 min. 5 sec.      | 38.0° C.     | 20 ml | 17l  |
|        | Bleaching         | 50 sec.            | 38.0° C.     | 5 ml  | 5l   |
|        | Fixing (1)        | 50 sec.            | 38.0° C.     | —     | 5l   |
|        | Fixing (2)        | 50 sec.            | 38.0° C.     | 8 ml  | 5l   |
|        | Washing           | 30 sec.            | 38.0° C.     | 17 ml | 3.5l |
|        | Stabilization (1) | 20 sec.            | 38.0° C.     | —     | 3l   |
| 15     | Stabilization (2) | 20 sec.            | 38.0° C.     | 15 ml | 3l   |
|        | Drying            | 1 min.30 sec.      | 60.0° C.     |       |      |

\* The quantity of replenisher is represented by a value per 1.1m of a 35-mm wide sample (equivalent to one 24 Ex. film).

The stabilizer was counterflowed from (2) to (1), and the overflow of washing water was entirely introduced to fixing (2). The fixer was also counterflow-piped from (2) to (1).

Note that the amounts of the developer, the bleaching solution, and the fixer carried over to the bleaching step, the fixing step, and the washing step were 2.5 ml, 2.0 ml, and 2.0 ml, respectively, per 1.1 m of a 35-mm wide light-sensitive material.

Note also that each crossover time was 6 sec, and this time was included in the processing time of each preceding step.

The aperture area of the processor was 100 cm<sup>2</sup> for the color developer, 120 cm<sup>2</sup> for the bleaching solution, and approximately 100 cm<sup>2</sup> for the other processing solutions.

The compositions of the processing solutions are presented below.

|    | (Color developer)                                           | Tank solution (g) | Replenishnent solution (g) |
|----|-------------------------------------------------------------|-------------------|----------------------------|
| 40 | Diethylenetriamine pentaacetic acid                         | 2.0               | 2.0                        |
|    | 1-hydroxyethylidene-1,1-diphosphonic acid                   | 2.0               | 2.0                        |
|    | Sodium sulfite                                              | 3.9               | 5.3                        |
| 45 | Potassium carbonate                                         | 37.5              | 39.0                       |
|    | Potassium bromide                                           | 1.4               | 0.4                        |
|    | Potassium iodide                                            | 1.3 mg            | —                          |
|    | Disodium-N,N-bis(sulfonate ethyl)hydroxylamine              | 8.0               | 11.0                       |
|    | 2-methyl-4-(N-ethyl-N-β-hydroxyethyl)amino)                 | 4.5               | 6.4                        |
| 50 | aniline sulfate                                             |                   |                            |
|    | Water to make                                               | 1.0l              | 1.0l                       |
|    | pH (adjusted by potassium hydroxide and sulfuric acid)      | 10.05             | 10.18                      |
|    | <u>(Bleaching solution)</u>                                 |                   |                            |
| 55 | Ferric ammonium 1,3-diaminopropanetetra acetate monohydrate | 118               | 180                        |
|    | Ammonium bromide                                            | 80                | 115                        |
|    | Ammonium nitrate                                            | 14                | 21                         |
| 60 | Succinic acid                                               | 40                | 60                         |
|    | Maleic acid                                                 | 33                | 50                         |
|    | Water to make                                               | 1.0l              | 1.0l                       |
|    | pH (adjusted by ammonia water)                              | 4.4               | 4.0                        |
|    | <u>(Fixer)</u>                                              |                   |                            |
| 65 | Ammonium methane sulfinate                                  | 10                | 30                         |

## 101

-continued

| (Color developer)                               | Tank solution (g) | Replenishment solution (g) |
|-------------------------------------------------|-------------------|----------------------------|
| Ammonium methane thiosulfonate                  | 4                 | 12                         |
| Aqueous ammonium thiosulfate solution (700 g/l) | 280 ml            | 840 ml                     |
| Imidazole                                       | 7                 | 20                         |
| Ethylenediamine tetraacetic acid                | 15                | 45                         |
| Water to make                                   | 1.0l              | 1.0l                       |
| pH (adjusted by ammonia water and acetic acid)  | 7.4               | 7.45                       |

## (Washing water)

Tap water was supplied to a mixed-bed column filled with an H type strongly acidic cation exchange resin (Amberlite IR-120B: available from Rohm & Haas Co.) and an OH type strongly basic anion exchange resin (Amberlite IR-400) to set the concentrations of calcium and magnesium to be 3 mg/l or less. Subsequently, 20 mg/l of sodium isocyanuric acid dichloride and 150 mg/l of sodium sulfate were added. The pH of the solution ranged from 6.5 to 7.5.

| (Stabilizer) common to tank solution and replenishment solution           | (g)  |
|---------------------------------------------------------------------------|------|
| Sodium p-toluenesulfinate                                                 | 0.03 |
| Polyoxyethylene-p-monononylphenylether (average polymerization degree 10) | 0.2  |
| Disodium ethylenediaminetetraacetate                                      | 0.05 |
| 1,2,4-triazole                                                            | 1.3  |
| 1,4-bis(1,2,4-triazole-1-ylmethyl) piperazine                             | 0.75 |
| 1,2-benzoisothiazoline-3-one                                              | 0.10 |
| Water to make                                                             | 1.0l |
| pH                                                                        | 8.5  |

The sharpness and color turbidity of each resultant sample were evaluated by the following methods.

## (Sharpness)

The sharpness was evaluated by a conventional MTF (Modulation Transfer Function) method. That is, MTF values at 10 cycles/mm of cyan and magenta images were obtained and represented by relative values assuming that the value of the sample 101 was 100.

## 102

Note that the MTF measurement was done by a method described in "Journal of Applied Photographic Engineering", Vol. 6(1), 1 to 8 (1980).

## 5 (Color turbidity)

The color turbidity of magenta with respect to a cyan density was evaluated in accordance with the following method.

(1) Double exposure was given to each sample as follows.

|    |                 |                                                                                                                                                                       |
|----|-----------------|-----------------------------------------------------------------------------------------------------------------------------------------------------------------------|
| 15 | First exposure  | Imagewise exposure was given with red light.                                                                                                                          |
| 20 | Second exposure | Uniform exposure was given to each sample with green light by an exposure amount by which the magenta density in a portion not exposed to red light of the sample 101 |
| 25 |                 | 1.7.                                                                                                                                                                  |

(2) Processing was performed by the same processing steps as described above.

(3) For each processed sample, a magenta density in a cyan-fogged portion was subtracted from a magenta density at a point at which a cyan density of 1.8 was given, and the obtained value was evaluated as the color turbidity.

The smaller the value, the lower the color turbidity and the higher the color saturation of a sensitive material.

The results are shown in TABLE 2.

TABLE 2

| Sample No. | Coupler in fourth layer  | Coupler in fifth layer   | Coupler in sixth layer   | MTF values   |                 |                 | Remarks             |
|------------|--------------------------|--------------------------|--------------------------|--------------|-----------------|-----------------|---------------------|
|            |                          |                          |                          | Cyan density | Magenta density | Color turbidity |                     |
| 101        | ExC-4                    | ExC-4                    | ExC-4                    | 100          | 100             | -0.23           | Comparative example |
| 102        | Comparative compound (1) | Comparative compound (1) | Comparative compound (1) | 99           | 98              | -0.26           | "                   |
| 103        | Comparative compound (2) | Comparative compound (2) | Comparative compound (2) | 97           | 97              | -0.24           | "                   |
| 104        | Comparative compound (3) | Comparative compound (3) | Comparative compound (3) | 94           | 94              | -0.20           | "                   |
| 105        | (1)                      | (1)                      | (1)                      | 106          | 106             | -0.30           | Present invention   |
| 106        | (2)                      | (2)                      | (2)                      | 107          | 106             | -0.30           | "                   |
| 107        | (3)                      | (3)                      | (3)                      | 106          | 106             | -0.29           | "                   |
| 108        | (10)                     | (10)                     | (10)                     | 107          | 106             | -0.30           | "                   |
| 109        | (12)                     | (12)                     | (12)                     | 107          | 107             | -0.30           | "                   |
| 110        | (35)                     | (35)                     | (35)                     | 106          | 106             | -0.30           | "                   |
| 111        | (44)                     | (44)                     | (44)                     | 107          | 106             | -0.30           | "                   |
| 112        | (44)                     | (44)                     | (1)                      | 107          | 106             | -0.29           | "                   |

103

As is apparent from the results shown in TABLE 2, when the compounds of the present invention were used the sharpness was significantly improved not only in the layer in which the compounds were used but also in other layers, and the color turbidity was also improved.

### Example 2

Samples 201 to 213 were formed by replacing the DIR compound ExY-1 in the eighth layer, ExY-1 and ExY-4 in the ninth layer, and ExY-1 in the twelfth layer of the sample 101 formed in Example 1 with comparative compounds (4), (5), and (6) presented below and the compounds of the present invention, and by controlling their addition amounts such that the gradation of the green-sensitive layer of each sample was equal to that of the sample 101. The sharpness of each resultant sample was evaluated by obtaining the MTF value at 10 cycles/mm of a magenta image following the same procedure as in Example 1. 15

the same procedure as in Example 1.  
Comparative compound (4): Compound (22) disclosed in  
IP-A-5-313322



Comparative compound (5): Compound (15) disclosed in  
JP-A-7-133259

104



### Comparative compound (6)



TABLE 3

| Sample No. | Coupler in eighth layer  | Coupler in ninth layer    | Coupler in twelfth layer | MTF value         |                     |
|------------|--------------------------|---------------------------|--------------------------|-------------------|---------------------|
|            |                          |                           |                          | (magenta density) | Remarks             |
| 101        | ExY-1                    | ExY-1, ExY-4              | ExY-1                    | 100               | Comparative example |
| 201        | Comparative compound (4) | Comparative compound (4)  | ExY-1                    | 97                | "                   |
| 202        | Comparative compound (5) | Comparative compound (5)  | ExY-1                    | 96                | "                   |
| 203        | Comparative compound (6) | Comparative *compound (6) | Comparative compound (6) | 95                | "                   |
| 204        | (16)                     | (16)                      | ExY-1                    | 108               | Present invention   |
| 205        | (18)                     | (18)                      | "                        | 108               | "                   |
| 206        | (23)                     | (23)                      | "                        | 109               | "                   |
| 207        | (24)                     | (24)                      | "                        | 108               | "                   |
| 208        | (34)                     | (34)                      | "                        | 106               | "                   |
| 209        | (45)                     | (45)                      | "                        | 108               | "                   |
| 210        | (48)                     | (48)                      | "                        | 107               | "                   |
| 211        | ExY-1                    | ExY-1, ExY-4              | (18)                     | 104               | "                   |
| 212        | (18)                     | (18)                      | (42)                     | 109               | "                   |
| 213        | (34)                     | (34)                      | (43)                     | 109               | "                   |

As can be seen from TABLE 3, a startling effect of improving the sharpness was obtained as in Example 1 even when the compounds of the present invention were used in green- and blue-sensitive layers.

#### Effect of the Invention

The present invention can provide a silver halide color photographic light-sensitive material which forms images having a high sharpness and a high color reproduction.

We claim:

1. A silver halide color photographic light-sensitive material containing a compound represented by formula (II) below:

Formula (II)



wherein A represents a coupler residue, Y represents an  $-SO_2R^1$ ,  $-SO_2NR_1R^2$ ,  $-CONR^1R^2$ ,  $-CO_2Z$ ,  $-CN$ ,  $-CF_3$ ,  $-CCl_3$ , or  $-NO_2$  group, and DI represents a development inhibitor residue which is bonded by a hetero atom and released to form mercaptoazole,

wherein each of  $R_1$  and  $R^2$  independently represents a hydrogen atom or a substituted or nonsubstituted alkyl, cycloalkyl, alkenyl, aryl, or heterocyclic group or  $R^1$  and  $R^2$  bond to each other to form a nitrogen-containing ring, and Z represents a hydrogen atom or a substituted or nonsubstituted cycloalkyl, alkenyl, aryl, or heterocyclic group.

2. The material according to claim 1, wherein Y is a  $-CONR^1R^2$ ,  $-CO_2Z$ ,  $-CN$ , or  $CF_3$  group.

3. The material according to claim 2, wherein Y is a  $-CN$  group.

4. The material according to claim 1, wherein said DI is represented by formulas DI-1 or DI-2 below:



40



45

wherein  $R_{91}$  represents a halogen atom, or a substituted or nonsubstituted alkyl, cycloalkyl, aryl, heterocyclic, alkoxy, cycloalkyloxy, aryloxy, heterocyclic oxy, silyloxy, acyloxy, alkoxy carbonyloxy, cycloalkyloxy carbonyloxy, aryloxy carbonyloxy, carbamoyloxy, sulfamoyloxy, alkanesulfonyloxy, arenesulfonyloxy, amide, alkanesulfonamide, arenesulfonamide, alkoxy carbonyl amino, cycloalkyloxy carbonyl amino, aryloxy carbonyl amino, ureido, nitro, acyl, alkoxy carbonyl, cycloalkyloxy carbonyl, aryloxy carbonyl, carbamoyl, cyano, alkylthio, arylthio, alkanesulfonyl, arenesulfonyl, alkoxy sulfonyl, cycloalkyloxy sulfonyl, aryloxy sulfonyl, or sulfamoyl group,

$R_{92}$  represents an alkyl, cycloalkyl, aryl, or heterocyclic group,

and V represents an oxygen atom, a sulfur atom, or  $-N(R_{93})-$  wherein  $R_{93}$  represents a group having the same meaning as  $R_{92}$ .

5. The material according to claim 1, wherein said coupler residue represented by A in formula (II) is coupler residue represented by formula (Cp-1), (Cp-2), (Cp-6), (Cp-7), (Cp-8), or (Cp-11) below, and said development inhibitor residue represented by DI in formula (II) is development inhibitor residue represented by formula (DI-1), (DI-2), or (DI-3) below,



## 107

-continued



DI-3

wherein R<sub>51</sub> represents an alkyl group, a cycloalkyl group, an aryl group, or a heterocyclic group, a represents 0 or 1, each of R<sub>52</sub> and R<sub>53</sub> independently represents a hydrogen atom, an alkyl group, a cycloalkyl group, an aryl group, or a heterocyclic group, and b represents 0 or 1, each of R<sub>58</sub> and R<sub>60</sub> independently represents an alkyl group, a cycloalkyl group, an aryl group, or a heterocyclic group, R<sub>59</sub> represents an alkyl group, a cycloalkyl group, an aryl group, a heterocyclic group, a silyl group, a carbonamide group, a sulfonamide group, an amino group, an anilino group, an alkylthio group, a cycloalkylthio group, an arylthio group, an alkoxy group, a cycloalkyloxy group, an aryloxy group, a ureido group, an alkoxy carbonylamino group, a cycloalkyloxycarbonylamino group, or a halogen atom, and d represents any integer from 0 to 3, if d is a plural number, a plurality of R<sub>59</sub>'s represent the same substituent group or different substituent groups, R<sub>61</sub> represents an alkyl group, a cycloalkyl group, an aryl group, a heterocyclic group, a carbamoyl group, an alkoxy carbonyl group, a cycloalkyloxycarbonyl group, an aryloxy carbonyl group, a cyano group, a sulfamoyl group, a carbonamide group, a ureido group, an alkoxy carbonylamino group, a cycloalkyloxycarbonylamino group, an aryloxy carbonylamino group, or a sulfonamide group, R<sub>62</sub> represents an alkyl group, a cycloalkyl group, an aryl group, a heterocyclic group, a carbonamide group, a sulfonamide group, an amino group, an anilino group, an alkylthio group, a cycloalkylthio group, an arylthio group, an alkoxy group, a cycloalkyloxy group, an aryloxy group, an alkoxy carbonylamino group, a cycloalkyloxycarbonylamino group, or a halogen atom, and e represents any integer from 0 to 4, if e is a plural number, a plurality of R<sub>62</sub>'s represent the same group or different groups, each of R<sub>64</sub> and R<sub>65</sub> independently represents a carbamoyl group, an alkoxy carbonyl group, a cycloalkyloxycarbonyl group, an aryloxy carbonyl group, a cyano group, a sulfamoyl group, an alkanesulfonyl group, an arenesulfonyl group, or a nitro group, R<sub>66</sub> represents a hydrogen atom, an alkyl group, a cycloalkyl group, an aryl group, or a heterocyclic group, wherein R<sub>91</sub> represents a halogen atom, or a substituted or nonsubstituted alkyl, cycloalkyl, aryl, heterocyclic, alkoxy, cycloalkyloxy, aryloxy, heterocyclic oxy, silyloxy, acyloxy, alkoxy carbonyloxy, cycloalkyloxycarbonyloxy,

## 108

aryloxy carbonyloxy, carbamoyloxy, sulfamoyloxy, alkanesulfonyloxy, arenesulfonyloxy, amide, alkane sulfonamide, arene sulfonamide, alkoxy carbonylamino, cycloalkyloxycarbonylamino, aryloxy carbonylamino, ureido, nitro, acyl, alkoxy carbonyl, cycloalkyloxycarbonyl, aryloxy carbonyl, carbamoyl, cyano, alkylthio, arylthio, alkanesulfonyl, arenesulfonyl, alkoxy sulfonyl, cycloalkyloxysulfonyl, aryloxy sulfonyl, or sulfamoyl group,

R<sub>92</sub> represents an alkyl, cycloalkyl, aryl, or heterocyclic group,

and V represents an oxygen atom, a sulfur atom, or —N(R<sub>93</sub>)— wherein R<sub>93</sub> represents a group having the same meaning as R<sub>92</sub>.

6. The material according to claim 5, wherein said coupler residue represented by A in formula (II) is coupler residue represented by formula (Cp-1) or (Cp-8), and said development inhibitor residue represented by DI in formula (II) is development inhibitor residue represented by (DI-1) or (DI-2).

7. The material according to claim 4, wherein R<sub>92</sub> is an alkyl, or aryl group.

8. The material according to claim 7, wherein R<sub>92</sub> is represented by —CH<sub>2</sub>CO<sub>2</sub>—R or —CH<sub>2</sub>CH<sub>2</sub>CO<sub>2</sub>—R, wherein R represents —C<sub>4</sub>—H<sub>9</sub>, —C<sub>5</sub>H<sub>11</sub>—n, —C<sub>5</sub>H<sub>11</sub>—i, —CH<sub>2</sub>CH=CHCH<sub>3</sub>, or —CH<sub>2</sub>CH=C(CH<sub>3</sub>)<sub>2</sub>.

9. The material according to claim 4, wherein V is an oxygen atom or sulfur atom, and R<sub>91</sub> is an alkylthio group or an arylthio group.

10. The material according to claim 9, wherein R<sub>91</sub> is represented by —SCH<sub>2</sub>CO<sub>2</sub>—R, —SCH<sub>2</sub>CH<sub>2</sub>CO<sub>2</sub>—R, or —SCH(CH<sub>3</sub>)CO<sub>2</sub>—R, wherein R has the same meaning as R<sub>92</sub>.

11. The material according to claim 4, wherein Y is a —CONR<sup>1</sup>R<sup>2</sup>, —CO<sub>2</sub>Z, —CN, or —CF<sub>3</sub> group.

12. The material according to claim 11, wherein Y is a —CN group.

13. The material according to claim 1, wherein each of R<sup>1</sup> and R<sup>2</sup> independently represents a hydrogen atom or a substituted or nonsubstituted alkyl group.

14. The material according to claim 13, wherein each of R<sup>1</sup> and R<sup>2</sup> independently represents a hydrogen atom or an alkyl group which has a hydroxyl group and/or a carboxyl group as a substituent and has 10 or less carbon atoms.

15. The material according to claim 1, wherein Z represents a hydrogen atom or a substituted or nonsubstituted aryl group.

16. The material according to claim 15, wherein Z represents a hydrogen atom or a substituted aryl group having 10 or less carbon atoms.

\* \* \* \* \*